



US012421665B2

(12) **United States Patent**  
**Creasey et al.**

(10) **Patent No.:** **US 12,421,665 B2**  
(45) **Date of Patent:** **\*Sep. 23, 2025**

(54) **PAPER ENHANCING COMPOSITIONS, USES THEREOF AND ENHANCED PAPER**

(71) Applicant: **ITI Technologies, Inc.**, Leland, NC (US)

(72) Inventors: **David H. Creasey**, Leland, NC (US); **Samuel Horace McCall, IV**, Leland, NC (US)

(73) Assignee: **ITI Technologies, Inc.**, Leland, NC (US)

(\*) Notice: Subject to any disclaimer, the term of this patent is extended or adjusted under 35 U.S.C. 154(b) by 210 days.

This patent is subject to a terminal disclaimer.

(21) Appl. No.: **18/223,816**

(22) Filed: **Jul. 19, 2023**

(65) **Prior Publication Data**

US 2023/0366154 A1 Nov. 16, 2023

**Related U.S. Application Data**

(60) Continuation-in-part of application No. 17/588,712, filed on Jan. 31, 2022, now Pat. No. 11,905,663, which is a division of application No. 16/896,328, filed on Jun. 9, 2020, now abandoned.

(51) **Int. Cl.**

**D21H 21/36** (2006.01)  
**D21H 17/67** (2006.01)  
**D21H 19/02** (2006.01)  
**D21H 19/38** (2006.01)  
**D21H 21/18** (2006.01)  
**D21H 21/24** (2006.01)  
**D21H 23/04** (2006.01)

(52) **U.S. Cl.**  
CPC ..... **D21H 21/36** (2013.01); **D21H 17/675** (2013.01); **D21H 19/02** (2013.01); **D21H 19/385** (2013.01); **D21H 21/18** (2013.01); **D21H 21/24** (2013.01); **D21H 23/04** (2013.01)

(58) **Field of Classification Search**  
CPC ..... D21H 17/67; D21H 17/675; D21H 19/02; D21H 19/36; D21H 19/38; D21H 19/385; D21H 21/18; D21H 21/24; D21H 21/36; D21H 23/04

See application file for complete search history.

(56) **References Cited**

**U.S. PATENT DOCUMENTS**

3,713,963 A 1/1973 Hager  
5,989,595 A 11/1999 Cummins  
RE41,109 E 2/2010 Cummins  
8,012,511 B1 9/2011 Cummins

(Continued)

**FOREIGN PATENT DOCUMENTS**

EP 2039829 A1 3/2009  
WO 9741302 A1 11/1997  
WO 2020210588 A1 10/2020

*Primary Examiner* — Jacob T Minskey

(74) *Attorney, Agent, or Firm* — E. Eric Mills; Nicholas P. Stadnyk; Maynard Nexsen PC

(57) **ABSTRACT**

The present invention provides certain paper enhancing compositions, typically aqueous compositions, for use in the manufacture and coating of paper, and paper products. The paper enhancing compositions provide certain paper processing advantages and distinct final paper product characteristics. The present invention further provides carbonate enhancing composition useful for preparing enhanced carbonate compositions used in the paper manufacturing processes.

**12 Claims, 6 Drawing Sheets**



(56)

**References Cited**

U.S. PATENT DOCUMENTS

|                 |         |                |
|-----------------|---------|----------------|
| 8,691,285 B2    | 4/2014  | Cummins        |
| 10,264,793 B2   | 4/2019  | Meccia         |
| 10,662,093 B2   | 5/2020  | Nicholas       |
| 2010/0126684 A1 | 5/2010  | Cheng          |
| 2017/0101740 A1 | 4/2017  | Harrington     |
| 2017/0280728 A1 | 10/2017 | Dautreuil      |
| 2019/0211508 A1 | 7/2019  | Creasey et al. |

Spectrograph - RT: 2.00-2.99



FIG. 1

Spectrograph -- RT: 2.01-2.99



FIG. 2

Spectrograph - RT: 2.00-2.98



FIG. 3

Spectrograph -- RT: 2.00-2.99



FIG. 4



FIG. 5



FIG. 6

## 1

PAPER ENHANCING COMPOSITIONS, USES  
THEREOF AND ENHANCED PAPERCROSS-REFERENCE TO RELATED  
APPLICATIONS

This application is a continuation-in-part application of U.S. patent application Ser. No. 17/588,712 filed on Jan. 31, 2022, which is a divisional application of U.S. patent Ser. No. 16/896,328 filed on Jun. 9, 2020 (now abandoned), which is related to U.S. patent application Ser. No. 16/745,846 entitled "Plastic Modifying Compositions and Enhanced Carbonate Compositions" filed on Jan. 17, 2020; the entire disclosures of which are incorporated herein by reference.

## BACKGROUND

The present invention relates to paper enhancing compositions useful for the manufacture of paper, paper products, paperboard and paperboard products, and coated paper and paperboard and products made therefrom including, for example and without limitation, cardboard and cardboard products. Also provided are enhanced carbonate compositions comprising at least one carbonate and at least one carbonate enhancing composition.

Although large-scale pulp-based paper processing methods have been established since the 1840's, a variety of substrates have been used and continue being used over the millennia including, for example and without limitation, cotton, silk, bamboo, *Phragmites* (e.g., common reeds) and traditional hard and soft wood sources. The use of such substrates each have particular challenges and techniques, and each typically use one or more fillers that extend the use of substrate(s), frequently reducing cost of the final product, while imparting specific and desired properties to the final product. Process development, particularly processes for continued cost reduction while maintaining and improving desired and/or new qualities to the final paper products continue. Accordingly, the present disclosure provides certain aspects relative to such continued development and improvement of a variety of products and processes for the processing of coated and uncoated paper and the coating of paper.

As further reviewed herein, once paper is manufactured, additional challenges exist when coating paper for a variety of uses. As such, the present invention also provides various aspects related to compositions and methods related to the preparation and processing of paper and paper products post manufacture of paper including, for example, a variety of coatings for various purposes.

## SUMMARY

One aspect of the present invention provides a paper forming mixture comprising a paper making fiber and at least one carbonate enhanced composition of the present invention. Addition of such carbonate enhanced mixture is typically, without limitation, added to the paper making process typically at the substrate slurry stage or at the wet-end stage although a carbonate enhanced composition can be added at any time prior to drying the paper.

Further provided is a paper forming mixture comprising a pulp-based mixture of pulp and/or other paper substrate and at least one carbonate enhanced composition of the present invention.

## 2

Also provided is a paper forming mixture comprising a paper making fiber and at least one paper enhancing composition of the present invention. Addition of such paper enhancing composition is added, among other uses as set forth herein, to the paper making process at the wet-end.

An additional aspect of the present invention provides a paper forming mixture comprising a pulp-based mixture of pulp and at least one carbonate enhanced composition of the present invention, wherein the amount of calcium carbonate 10 filler is at least five percent (5%) greater than the amount calcium carbonate fill typically added to a given paper type. For example, and without limitation, as reviewed in part above, for a paper type typically using 10-30% fill, the amount of fill that can be added to the paper forming wet 15 mixture will equal at least 31.5% of the total wet mixture. This increase in calcium carbonate fill amount can be used for any paper type well known to the skilled artisan.

Another aspect of the present invention provides for enhanced carbonate compositions comprising the addition 20 of a carbonate enhancing composition to carbonate, typically calcium carbonate, or another filler material.

A further aspect of the present invention provides for a method of modifying the zeta potential of calcium carbonate used in a paper making process comprising the addition of 25 at least one carbonate enhanced composition of the present invention to the wet-end of a paper making process. As used relative to the zeta potential, such modification can be an increase or decrease of the zeta potential, but typically is an increase in the zeta potential as used herein.

More particularly, the present invention also provides a 30 method of modifying the zeta potential of calcium carbonate used in a pulp- or other paper substrate-based paper making processes comprising the addition of at least one carbonate enhanced composition of the present invention to the substrate slurry and/or wet-end stage of a paper making process.

An additional aspect of the present invention provides for 35 antimicrobial paper, having a multitude of uses, comprising paper prepared by the addition of at least one carbonate enhanced composition of the present invention to the substrate slurry stage and/or wet-end stage of a paper making process. As used herein, the term "antimicrobial activity" means the inhibition of microbes.

The present invention further provides a paper enhancing 40 composition comprising water, at least one solubility enhancing aqueous composition, sodium hydroxide, copper and/or silver sulfate and, optionally, at least one surfactant selected from the group consisting of non-ionic surfactants and/or anionic surfactants.

An additional aspect of the present invention provides an 45 aqueous or, substantially aqueous, paper enhancing composition (aqueous notwithstanding the potential for copper sulfate and/or silver sulfate to not have completely dissolved in the paper enhancing composition) comprising an aqueous phase comprising a solubility enhancing aqueous composition 50 wherein 1 part of a first solution is added to about 15 to about 20 parts of water, frequently deionized water, to form a second solution; dilute sodium hydroxide solution (sodium hydroxide concentration from about 20 percent to about 50 percent dilution) having a concentration of about 5% to about 7.5% weight/weight of the total aqueous phase weight of the composition; at least one surfactant selected from the group 55 consisting of non-ionic surfactants and anionic surfactants having a concentration from about 0.05 percent to about 0.15 percent weight/weight of the total aqueous phase weight of the composition; and copper sulfate having a concentration from about 20 percent to about 26 percent weight/weight of the total aqueous phase weight of the

composition. As used herein, the term "aqueous paper enhancing composition" also includes any such composition that is substantially aqueous as indicated herein.

Another aspect provides for a paper enhancing composition wherein silver sulfate is included in addition to or in lieu of the copper sulfate at a concentration from about 0.001 percent to about 1.5 percent weight/weight of the total aqueous phase weight of such composition.

A further aspect of the present invention further comprises the addition of an acid or base to adjust the pH to a pH from about 2.5 to about 3.5 to a paper enhancing composition of the present invention.

An additional aspect of the present invention provides an aqueous paper enhancing composition comprising a solubility enhancing aqueous composition comprising an anionic component comprising sulfate ions, alone or in combination with bisulfate ions, having a concentration from about 8.00 moles per liter to about 13.00 moles per liter of the solubility enhancing composition volume, a cationic component comprising ammonium ions having a concentration from about 1.45 moles per liter to about 2.01 moles per liter of the solubility enhancing composition volume, and a hydrogen ion component in a concentration from about 17.38 to about 21.68 moles per liter of the total volume of the solubility enhancing composition solution; a dilute sodium hydroxide solution (about 20% to about 50% dilution) having a concentration of about 5 percent to about 7.5 percent weight/weight of the total aqueous phase weight of the paper enhancing composition; at least one optional surfactant selected from the group consisting of non-ionic surfactant and anionic surfactant having a concentration from about 0.05 percent to about 0.15 percent weight/weight of the total aqueous phase weight of the paper enhancing composition; and silver sulfate having a concentration from about 0.001 percent to about 1.5 percent weight/weight of the total aqueous phase weight of the paper enhancing composition. This present aspect of the invention is also provided without copper sulfate and/or silver sulfate.

A further aspect of the present invention further comprises the addition of an acid or base to adjust the pH to a pH from about 2.5 to about 3.5 to the immediately two preceding compositions.

An addition aspect of the present invention provides a paper enhancing composition consisting of: a solubility enhancing composition comprising an anionic component comprising sulfate ions, alone or in combination with bisulfate ions, having a concentration from about 8.00 moles per liter to about 13.00 moles per liter of the solubility enhancing composition volume, a cationic component comprising ammonium ions having a concentration from about 1.45 moles per liter to about 2.01 moles per liter of the solubility enhancing composition volume, and a hydrogen ion component in a concentration from about 17.38 to about 21.68 moles per liter of the total volume of the solubility enhancing composition; a dilute sodium hydroxide solution having a concentration of about 5 percent to about 7.5 percent weight/weight of the total aqueous phase weight of the paper enhancing composition wherein the dilute sodium hydroxide solution has a concentration from about 20 percent to about 50 percent sodium hydroxide; at least one surfactant selected from the group consisting of non-ionic surfactant and anionic surfactant having a concentration from about 0.05 percent to about 0.15 percent weight/weight of the total aqueous phase weight of the paper enhancing composition; silver sulfate having a concentration from about 0.001 percent to about 1.5 percent weight/weight of the total weight of the paper enhancing composition; and at least one

acid or at least one base to adjust the final pH of the paper enhancing composition in a range from about pH 2.5 to about pH 3.5.

The present invention further provides a method of increasing at least one of the group consisting of paper tensile, bond and burst strength of paper comprising the addition of at least one paper enhancing composition of the present invention to during or following the paper making process (e.g., a paper coating) compared to a paper making process not using such paper enhancing composition.

The present invention also provides a method of increasing at least one of paper tensile strength, bond strength and burst strength compared to paper prepared without the addition of at least one paper enhancing composition comprising the addition of at least one paper enhancing composition to a substrate slurry stage or to the wet-end stage of the paper making process.

Another aspect of the present invention provides a method for decreasing the interstitial pore size between and among paper fibers in a wet-end-paper making process compared to paper prepared without the addition of at least one paper enhancing composition comprising the addition of at least one paper enhancing composition to the substrate slurry stage or wet-end stage of the paper making process.

An additional aspect of the present invention provides a method for increasing paper density compared to paper prepared without the addition of at least one paper enhancing composition comprising the addition of at least one paper enhancing composition to the substrate slurry stage or wet-end stage of the paper making process.

A further aspect of the present invention provides for paper having antimicrobial properties comprising paper prepared using at least one paper enhancing composition during the paper making process or afterward (e.g., as a paper coating or as one aspect of a paper coating).

Also provided herein is a method of modifying the zeta potential of calcium carbonate when used in the paper making process comprising adding at least one aqueous carbonate enhancing composition to calcium carbonate or other fill material prior to the introduction of such calcium carbonate or other fill material to the paper making process as further described herein.

Another aspect of the present invention provides for enhanced paper comprising paper having applied to such paper at least one aqueous enhancing paper composition during any stage of the paper making process or afterward (e.g., as a paper coating or as one aspect of a paper coating).

Further provided herein are the following methods:

A method of enhancing paper comprising applying at least one aqueous paper enhancing composition during any stage of the paper making process or afterward (e.g., as a paper coating or as one aspect of a paper coating).

A method of increasing at least one of the group consisting of tensile strength, bond strength and burst strength in paper compared to the respective tensile strength, bond strength and burst strength of paper untreated with an aqueous paper enhancing composition comprising applying at least one aqueous paper enhancing composition during any stage of the paper making process or afterward (e.g., as a paper coating or as one aspect of a paper coating).

A method of increasing at least one of the group consisting of paper tensile strength, bond strength and burst strength of paper comprising applying at least one aqueous paper enhancing composition during any stage of paper production, typically the wet-end stage, com-

pared to paper untreated with an aqueous paper enhancing composition without an increase in caliper pose.

Further provided is antimicrobial paper, having a multitude of uses, comprising paper prepared by the application of at least one aqueous paper enhancing composition of the present invention during any stage of paper production including, for example and without limitation, a paper coating stage.

Another aspect of the present invention provides for a paper coating comprising at least one aqueous paper enhancing composition.

An additional aspect provides for paper coated with at least one aqueous paper enhancing composition.

Another aspect of the present invention provides a method of increasing at least one of the group consisting of paper tensile strength, bond strength and burst strength of paper comprising the application of a coating to paper comprising at least one paper enhancing composition of the present invention.

An additional aspect of the present invention provides for a method of providing at least one of protection from fingerprints and other blemishes, help prevent metallic inks from tarnishing, and provide paper surfaces that can be written on with multiple media (including, without limitation, pencil, pen, ink jet printers, laser jet printers off-set printers and the like) comprising the application of a coating to paper comprising at least one paper enhancing composition of the present invention.

A further aspect of the present invention provides for a method of providing improvement of at least one of protection from fingerprints and other blemishes, help prevent metallic inks from tarnishing, and provide paper surfaces that can be written on with multiple media (including, without limitation, pencil, pen, ink jet printers, laser jet printers off-set printers and the like) compared to paper coatings not including the application of at least one aqueous paper enhancing composition of the present invention comprising the application of a coating to paper comprising at least one paper enhancing composition of the present invention.

Accordingly, another aspect of the present invention provides for coated paper having antimicrobial activity comprising paper coated with at least one aqueous paper enhancing composition of the present invention.

An additional aspect of the present invention provides for paper having antimicrobial properties comprising paper made with or coated with at least one aqueous paper enhancing composition of the present invention.

Another aspect of the present invention provides for a method of preparing paper having antimicrobial activity comprising applying as a coating to paper at least one aqueous paper enhancing composition of the present invention to said paper.

Another aspect of the present invention provides a method of extending the shelf-life of perishable foodstuff comprising placing such foodstuff in contact with paper made with and/or coated with at least one aqueous paper enhancing composition of the present invention. Such shelf-life can be extended for at least 24 hours compared to a paper product that was untreated with a paper enhancing composition, providing substantial value to providers of such perishable foodstuff.

Further provided is a method for preparing paper for medical and industrial protective uses comprising applying as a coating to paper at least one aqueous paper enhancing composition.

An additional aspect provides a method of preparing paper for use in masks for mammalian, particularly human, use comprising applying as a coating at least one aqueous paper enhancing composition.

5 An additional aspect of the present invention provides a carbonate enhanced composition comprising at least one carbonate or other fill material and at least one carbonate enhancing composition.

10 A further aspect of the present providers a carbonate enhancing composition which is the same as each paper enhancing composition as taught herein. These compositions differ in their uses wherein paper enhancing compositions are used as described herein whereas carbonate enhancing compositions are used to prepare enhanced carbonate compositions or for enhancing other fill materials, also as further described herein.

15 Another aspect of the present invention provides for a carbonate enhancing composition consisting of: a solubility enhancing composition comprising an anionic component comprising sulfate ions, alone or in combination with bisulfate ions, having a concentration from about 8.00 moles per liter to about 13.00 moles per liter of the solubility enhancing composition volume, a cationic component comprising ammonium ions having a concentration from about 1.45 moles per liter to about 2.01 moles per liter of the solubility enhancing composition volume, and a hydrogen ion component in a concentration from about 17.38 to about 21.68 moles per liter of the total volume of the solubility enhancing composition; a dilute sodium hydroxide solution having a concentration of about 5 percent to about 7.5 percent weight/weight of the total aqueous phase weight of the paper enhancing composition wherein the dilute sodium hydroxide solution has a concentration from about 20 percent to about 30 percent sodium hydroxide; at least one surfactant selected from the group consisting of non-ionic surfactant and anionic surfactant having a concentration from about 0.05 percent to about 0.15 percent weight/weight of the total aqueous phase weight of the paper enhancing composition; 20 silver sulfate having a concentration from about 0.001 percent to about 1.5 percent weight/weight of the total weight of the paper enhancing composition; and at least one acid or at least one base to adjust the final pH of the paper enhancing composition in a range from about pH 2.5 to about pH 3.5.

25 Other aspects of the present invention provide a variety of methods of using a carbonate enhanced composition of the present invention to a variety of intermediate and final products as further described herein below.

30 An additional aspect of the present invention provides a carbonate enhancing composition comprising an aqueous phase comprising a solubility enhancing aqueous composition wherein 1 part of a first solution is added to about 15 to about 20 parts of water to form a second solution; sodium hydroxide solution having a concentration of about 5% to about 7.5% weight/weight of the total aqueous phase weight of the carbonate enhancing composition; at least one surfactant selected from the group consisting of non-ionic surfactants and anionic surfactants having a concentration from about 0.05 percent to about 0.15 percent weight/weight of the total aqueous phase weight of the carbonate enhancing composition; and copper sulfate having a concentration from about 20 percent to about 26 percent weight/weight of the total aqueous phase weight of the carbonate enhancing composition; optionally comprising the addition of at least one acid or at least one base to adjust the final composition pH to a pH of about 2.5 to about 3.5.

Another aspect of the present invention provides a carbonate enhancing composition comprising an aqueous phase comprising a solubility enhancing aqueous composition wherein 1 part of a first solution is added to about 15 to about 20 parts of water to form a second solution and sodium hydroxide solution having a concentration of about 5% to about 7.5% weight/weight of the total aqueous phase weight of the composition; and copper sulfate having a concentration from about 20 percent to about 26 percent weight/weight of the total aqueous phase weight of the composition, optionally comprising the addition of at least one acid or at least one base to adjust the final composition pH to a pH of about 2.5 to about 3.5.

An additional aspect of the present invention provides an antimicrobial composition comprising at least one composition selected from the group consisting of at least one carbonate enhanced composition and at least one carbonate enhancing composition, wherein the carbonate enhancing composition is optionally aqueous or substantially aqueous.

A further aspect of the present invention provides a product requiring at least one carbonate as an element in the manufacture thereof comprising at least, in part, one carbonate enhanced composition used in the manufacture of such product.

An additional aspect of the present invention provides an antimicrobial composition comprising at least one carbonate enhanced composition.

#### BRIEF DESCRIPTION OF THE DRAWINGS

Features of the present invention will be more fully appreciated by reference to the following detailed description when taken in conjunction with the following drawings in which:

FIG. 1. depicts a low resolution spectrogram with 1 part reaction unit to 5 parts total.

FIG. 2. depicts a high resolution spectrogram with 1 part reaction unit to 5 parts total.

FIG. 3. depicts a low resolution spectrogram with 1 part reaction unit to 10 parts total.

FIG. 4. depicts a high resolution spectrogram with 1 part reaction unit to 10 parts total.

FIG. 5. depicts a low resolution spectrogram with 1 part reaction unit to 20 parts total.

FIG. 6. depicts a high resolution spectrogram with 1 part reaction unit to 20 parts total.

Each of the spectrograms was run according to the respective teachings of Example 6. Each of the spectrograms depicts compositions that are free of salt crystals or other solids formed from the ammonium sulfate and sulfuric acid reactants.

While the aspects of the present disclosure are susceptible to various modifications and alternative forms, specific embodiments thereof are shown by way of example in the drawings and will herein be described in detail. It should be understood, however, that the drawings and detailed description are not intended to limit the disclosure to the particular forms illustrated but, on the contrary, the intention is to cover all modifications, equivalents and alternatives falling within the spirit and scope of the present disclosure as defined by the appended claims. The headings used herein are used for organizational purposes only and are not meant to limit the scope of the description. As used throughout this application, the word "may" is used in a permissive sense, meaning: "having the potential to"; rather than the mandatory sense meaning: "must". Similarly, the words "include", "including" and "includes" means including, without limita-

tation. Additionally, as used in this specification and the appended claims, the singular forms "a", "an" and "the" include singular and plural referents unless the content clearly dictates otherwise.

5 The scope of the present disclosure includes any feature or combination of features disclosed herein (either explicitly or implicitly), or any generalization thereof, whether or not it mitigates any or all of the problems addressed herein. Accordingly, new claims may be formulated during prosecution of this application (or an application claiming priority thereto) to any such combinations of features. In particular, with reference to the appended claims, features from dependent claims may be combined with those of independent claims and features from respective independent claims may be combined in any appropriate manner and not merely in the specific combinations enumerated in the appended claims.

#### DETAILED DESCRIPTION

##### Definitions

The term "antimicrobial" means antibacterial, anti-fungal, antiviral and anti-mold, each individually and collectively.

The term "alkali and alkaline metal carbonates" have their traditional meanings in the art.

The term "calcium carbonate" has its traditionally meaning and included, for example and without limitation, ground calcium carbonate, precipitated calcium carbonate and needle calcium carbonate, each being prepared in a variety of, for example and without limitation, purities, densities, fineness of grain, morphologies, surface areas, high oil absorption, bulk densities from ultra-low to super high powder densities, and the like.

The term "carbonate enhancing composition" as taught herein is synonymous with the term "paper enhancing composition", also as taught herein. Although the compositions and the benefits to intermediate and final paper products are the same, the former is added to a carbonate or other filler material prior to such filler material being added to a pulp slurry; whereas the latter can be added anywhere during the paper forming process, as further described herein, or to a paper product after drying and forming. As such, the two terms are interchangeable relative to the preparation, use and benefits of the respective term, differentiated by the respective use of the respective composition.

The term "dilute sodium hydroxide" means sodium hydroxide, typically but not limited to solid form, diluted with water to a concentration of greater than about 20 percent.

The term "first solution" means a solution of ammonium sulfate and sulfuric acid as further described herein and used in preparing a solubility enhancing aqueous composition.

The term "fill material", "filler" or "fill" means at least 55 one of calcium carbonate, chalk, clay including for example and without limitation China clay, talc, titanium dioxide and/or one or more other natural or synthetic material that is typically added to a substrate or paper forming mixture which typically includes pulp or other substrate material, 60 with or without the addition of other additives used in the paper industry, for the formation of a final paper product which includes, for example and without limitation, calcium carbonate. The term "fill material", when used more generally in reference to the enhanced carbonate compositions of 65 the present invention, has the traditional meaning as used in the art for the respective product in which the enhanced carbonate composition is used. Fill material added during

the paper making process is measured and used on a mass/mass (or weight/weight) basis relative to relative to the mass of a pulp slurry to which the fill material is added.

The term "free of solids" means that the solubility enhancing aqueous composition do not form salt crystals or other solids that remain in the composition over time, such salt crystals or other solids being formed from the reactants of ammonium sulfate and sulfuric acid and other elements of a paper enhancing composition.

The term "fiber" means at least one or a group or mass of pulp and/or other paper making substrate used in the paper making process. Inherent in this definition is the term "pulp fiber".

The term "inhibition" or "inhibiting" means the act of prophylaxis, retarding and/or controlling the growth of microbes in products as described herein.

The term "microbes" means, individually or collectively, bacteria, fungi, viruses and/or mold.

The term "paper" means paper, paperboard (single or multi-ply) and other known paper-based products, unless otherwise differentiated, as each term is known in the art.

The term "paper, paperboard product(s), linerboard and tissue" means, without limitation, any paper based product that contains or is made from paper, paperboard, linerboard and/or tissue, in part or in whole. One example of such products includes, without limitation, cardboard. Such products can be intermediate products that are subjected to further processing and/or final products used by an end user.

The term "pulp" or "paper pulp" (used interchangeably) means any raw material or combination of raw materials used for paper manufacture. Paper pulp or pulp can contain, for example and without limitation, vegetable, cellulosic, mineral and/or man-made fibers. Individually or collectively, as used herein, the terms "pulp" and "paper pulp" are also referred to herein as a "substrate".

The term "paper substrate" means for example and without limitation, cotton, silk, bamboo, *Phragmites* (e.g., common reeds) and traditional hard and soft wood sources.

The term "reaction unit" relative to the preparation of a solubility enhancing aqueous composition means the desired total volume of a first solution as expressed as a ratio of a range of ammonium sulfate concentrations to sulfuric acid concentrations (the reactants).

The term "second solution" means the first solution as prepared for a final volume plus the requisite amount of water to form a composition of the present invention as further described herein and used in preparing a solubility enhancing aqueous composition.

The term "sodium hydroxide solution" means a sodium hydroxide, typically in a dilute sodium hydroxide solution, wherein the solution can be any dilution as further set forth herein.

The term "solubility enhancing aqueous composition" means the solubility enhancing aqueous compositions as described herein.

The term "starch" has the meaning generally known and accepted in the paper manufacturing art and as generally reviewed in *Starch* (Third Edition), Chemistry and Technology, Food Science and Technology 2009, Pages 657-713.

The term "sulfate anions" encompasses each of sulfate anions, bisulfate anions and combinations thereof. Combinations of sulfate anions and bisulfate anions are common in the solubility enhancing aqueous compositions described herein.

The term "sulfuric acid" means concentrated sulfuric acid having a concentration of from about 95% to about 98%.

The term "substantially free of solids" means that the solubility enhancing aqueous compositions and/or the enhanced carbonate compositions described herein are at least 95 percent aqueous or, alternatively, at least 98 percent aqueous without the formation of salt crystals or other solids. The addition of materials not an element of the solubility enhancing aqueous compositions and/or paper enhancing compositions and/or carbonate enhancing compositions in the preparation of compositions of the present invention may affect the amount of salts and/or other solids. As such, the term "substantially free of solids" pertains only to the preparations of each of the solubility enhancing aqueous compositions, paper enhancing compositions and carbonate enhancing compositions of the present invention described herein.

## DESCRIPTION

The following description and examples are included to demonstrate the embodiments of the present disclosure. It should be appreciated by those of skill in the art that the compositions, techniques and methods disclosed in the examples herein function in the practice of the disclosed embodiments. However, those skilled in the respective arts should, in light of the present disclosure, appreciate that changes can be made to the specific embodiments and still obtain a like or similar result without departing from the spirit and scope of the disclosed embodiments.

Solutions to multiple well-known and long-standing problems in the paper manufacturing industry are provided herein. Paper manufacturers are continually seeking to reduce the cost of paper manufacture. It is well known in the industry that paper substrate (e.g., pulp) is substantially more costly than the second largest mass/weight component, fill material (e.g., calcium carbonate). As such, manufacturers have been attempting to increase the amount of fill material used while decreasing the amount of substrate used. It is well known in the art that an increase in fill material can result in for example, decreases in strength, higher frequencies of web breaks, increased apparent density, low first pass retention and potential abrasion to slitter knives and die cutters. Each of these problems are addressed by the use of the compositions taught herein along with addressing other problems as set forth herein.

Addressed further hereinbelow is the additional issue of using silver sulfate in paper forming mixtures wherein the resulting intermediate and/or final product(s) are turned irretrievably black from the improper use of silver sulfate.

The present specification includes references to "one aspect/embodiment" or "an aspect/embodiment". These phrases do not necessarily refer to the same embodiment although embodiments that include any combination of the features or elements disclosed herein are generally contemplated unless expressly disclaimed herein. Particular features, processes, elements or characteristics may be combined in any suitable manner consistent with this disclosure.

With the pulp-paper industry, at least three additional well-known and long-standing problems exist with the use of calcium carbonate filler (e.g., precipitated, ground, needles and, without limitation, the like) incorporated into the paper making process, typically added to a substrate slurry or afterward, particularly increased use of such filler: i. filler particles added to fiber suspended in water are not easily retained in the forming sheet because they are often too small to be entrapped mechanically and because filler particles are negatively charged, they repel each other; ii. filler particles can interfere with fiber-fiber bonding; there-

## 11

fore, causing tensile strength of the paper to suffer; and iii. the addition of calcium carbonate beyond a certain level will cause, among other problems, reduced paper strength and stiffness, increased size demand, and increased abrasion and dusting.

Moreover, there are four primary means by which filler, particularly calcium carbonate, interacts with pulp fiber: i. calcium carbonate is distributed among the fibers; ii. one end of calcium carbonate is embedded in one fiber with the other end embedded in another fiber; iii. one end of calcium carbonate is embedded in one fiber with the other end being distributed among the fibers; and iv. calcium carbonate is entirely embedded in a fiber. The challenge is to provide for an environment for fiber-filler entanglement and friction while also providing for enhanced hydrogen bonding. The potential benefits can be an increase in filler loading, reducing fiber/substrate input and reducing paper costs, while maintaining the positive attributes typical of calcium carbonate used as a filler in paper, which are many and well known in the art.

Although filler particles (type and size) are frequently designed to accommodate individual paper customer needs, there exists a wide range of filler introduced during this aspect of the paper making process. For example, and without limitation, calcium carbonate filler is generally about 10% to about 30%, typically about 20% for printing paper. The introduction of calcium carbonate can be added during the substrate slurry stage, at the wet-end stage or as a surface application. Filler level of up to about 50%, although not common, can be used for coated papers (e.g., wood-free 135 g/m<sup>2</sup>) and copy and office paper (75-80 g/m<sup>2</sup> with up to 30% filler used; although 15% filler is reported to be used in North America for weight levels up to 75 g/m<sup>2</sup>). In essence, there are a plethora of variables known in the paper preparation art which are incorporated into a variety of processes, including numerous forms of filler, particularly calcium carbonate, used to form a broad range of paper products. It is not the intent of this disclosure to reteach paper making processes. Rather, it is the intent to recite a representative sample of some of the processes, and related variables, used in an intricate yet well-known art. As such, the use of calcium carbonate and, more specifically, carbonate enhanced compositions of the present disclosure, is not to be limited to the brief review of paper making processes disclosed herein. In fact, the carbonate enhanced compositions of the present invention can be used in lieu of straight calcium carbonate regardless of form, as used in wet-end processing.

Without being held to a particular theory, it is believed that the addition of at least one carbonate enhanced composition of the present invention compared to using straight calcium carbonate as a filler in pulp-based or other paper making processes modifies the zeta potential of the calcium carbonate, potentially providing stronger bonds/interaction between the fiber and calcium carbonate filler. The end result is a potentially higher percentage of calcium carbonate in the wet-end without the negative attributes associated with increased amounts of filler for each particular paper type. Such use of carbonate enhanced compositions of the present invention provides, without limitation, excellent runnability, overall potential cost savings, improved hydrophobic sizing, opacity, and print characteristics, and improved, or at least not a loss, of tensile, bond and/or burst strength, while potentially not affecting paper caliper or caliper pose compared to the use of non-enhanced calcium carbonate.

One aspect of the present invention provides a paper forming mixture comprising a paper making fiber and at

## 12

least one carbonate enhanced composition of the present invention. Addition of such carbonate enhanced mixture is typically, without limitation, added to the paper making process typically at the substrate slurry stage or at the 5 wet-end stage although a carbonate enhanced composition can be added at any time prior to drying the paper.

Further provided is a paper forming mixture comprising a pulp-based mixture of pulp and/or other paper substrate and at least one carbonate enhanced composition of the present 10 invention.

Also provided is a paper forming mixture comprising a paper making fiber and at least one paper enhancing composition of the present invention. Addition of such paper enhancing composition is added, among other uses as set 15 forth herein, to the paper making process at the wet-end.

An additional aspect of the present invention provides a paper forming mixture comprising a pulp-based mixture of pulp and at least one carbonate enhanced composition of the present invention, wherein the amount of calcium carbonate 20 filler is at least five percent (5%) greater than the amount calcium carbonate fill typically added to a given paper type. For example, and without limitation, as reviewed in part above, for a paper type typically using 10-30% fill, the amount of fill that can be added to the paper forming wet 25 mixture will equal at least 31.5% of the total wet mixture.

Moreover, the paper industry has been seeking means by which to significantly increase the amount of fill material for decades, resulting in a substantial cost savings, without negatively impacting the resulting paper quality. The present 30 enhanced carbonate and paper forming compositions of the present invention allow for increases of fill material, typically calcium carbonate, of at least 40 percent and in a range of up to 70% for paper which is intended to disintegrate (e.g. toilet paper). As such, fill material treated with enhanced 35 carbonate compositions of the present invention resulting in enhanced carbonate compositions of the present invention can be used at a concentration of 40%, 50%, 60% and 70%, or any whole number or fraction within the stated range, relative to the paper making material to which the enhanced 40 carbonate compositions are added, typically on a weight/weight basis.

Another aspect of the present invention provides for enhanced carbonate compositions comprising the addition of a carbonate enhancing composition to carbonate, typically calcium carbonate, or another filler material.

A further aspect of the present invention provides for a method of modifying the zeta potential of calcium carbonate used in a paper making process comprising the addition of at least one carbonate enhanced composition of the present 50 invention to the wet-end of a paper making process. As used relative to the zeta potential, such modification can be an increase or decrease of the zeta potential, but typically is an increase in the zeta potential as used herein.

More particularly, the present invention also provides a 55 method of modifying the zeta potential of calcium carbonate used in a pulp- or other paper substrate-based paper making processes comprising the addition of at least one carbonate enhanced composition of the present invention to the substrate slurry and/or wet-end stage of a paper making process.

As taught herein, the addition of a carbonate enhanced 60 composition and/or a paper enhanced composition of the present invention, through the modification of carbonate zeta potential and otherwise, has the potential to form more and tighter bonds among the fiber and fill material than is otherwise typically the case when using only unenhanced calcium carbonate as a fill material rather than at least one carbonate enhanced composition of the present invention or

the use of a paper enhancing composition of the present invention. As such, the pores of the paper can be reduced with the use of the carbonate enhanced composition resulting in paper that is less penetrable to dust and other particulate matter, pollutants and microorganisms.

An additional aspect of the present invention provides for antimicrobial paper, having a multitude of uses, comprising paper prepared by the addition of at least one carbonate enhanced composition of the present invention to the substrate slurry stage and/or wet-end stage of a paper making process. As used herein, the term "antimicrobial activity" means the inhibition of microbes.

The present invention further provides a paper enhancing composition comprising water, at least one solubility enhancing aqueous composition, sodium hydroxide, copper and/or silver sulfate and, optionally, at least one surfactant selected from the group consisting of non-ionic surfactants and/or anionic surfactants.

An additional aspect of the present invention provides an aqueous or, substantially aqueous, paper enhancing composition (aqueous notwithstanding the potential for copper sulfate and/or silver sulfate to not have completely dissolved in the paper enhancing composition) comprising an aqueous phase comprising a solubility enhancing aqueous composition wherein 1 part of a first solution is added to about 15 to about 20 parts of water, frequently deionized water, to form a second solution; dilute sodium hydroxide solution (sodium hydroxide concentration from about 20 percent to about 50 percent dilution) having a concentration of about 5% to about 7.5% weight/weight of the total aqueous phase weight of the composition; at least one surfactant selected from the group consisting of non-ionic surfactants and anionic surfactants having a concentration from about 0.05 percent to about 0.15 percent weight/weight of the total aqueous phase weight of the composition; and copper sulfate having a concentration from about 20 percent to about 26 percent weight/weight of the total aqueous phase weight of the composition. As used herein, the term "aqueous paper enhancing composition" also includes any such composition that is substantially aqueous as indicated herein.

Another aspect provides for a paper enhancing composition wherein silver sulfate is included in addition to or in lieu of the copper sulfate at a concentration from about 0.001 percent to about 1.5 percent weight/weight of the total aqueous phase weight of such composition.

A further aspect of the present invention further comprises the addition of an acid or base to adjust the pH to a pH from about 2.5 to about 3.5 to a paper enhancing composition of the present invention.

An additional aspect of the present invention provides an aqueous paper enhancing composition comprising a solubility enhancing aqueous composition comprising an anionic component comprising sulfate ions, alone or in combination with bisulfate ions, having a concentration from about 8.00 moles per liter to about 13.00 moles per liter of the solubility enhancing composition volume, a cationic component comprising ammonium ions having a concentration from about 1.45 moles per liter to about 2.01 moles per liter of the solubility enhancing composition volume, and a hydrogen ion component in a concentration from about 17.38 to about 21.68 moles per liter of the solubility enhancing composition solution; a dilute sodium hydroxide solution (about 20% to about 50% dilution) having a concentration of about 5 percent to about 7.5 percent weight/weight of the total aqueous phase weight of the paper enhancing composition; at least one optional surfactant selected from the group consisting of non-ionic

surfactant and anionic surfactant having a concentration from about 0.05 percent to about 0.15 percent weight/weight of the total aqueous phase weight of the paper enhancing composition; and silver sulfate having a concentration from about 0.001 percent to about 1.5 percent weight/weight of the total aqueous phase weight of the paper enhancing composition. This present aspect of the invention is also provided without copper sulfate and/or silver sulfate.

A further aspect of the present invention further comprises the addition of an acid or base to adjust the pH from about 2.5 to about 3.5 to the immediately two preceding compositions.

An addition aspect of the present invention provides a paper enhancing composition consisting of: a solubility enhancing composition comprising an anionic component comprising sulfate ions, alone or in combination with bisulfate ions, having a concentration from about 8.00 moles per liter to about 13.00 moles per liter of the solubility enhancing composition volume, a cationic component comprising ammonium ions having a concentration from about 1.45 moles per liter to about 2.01 moles per liter of the solubility enhancing composition volume, and a hydrogen ion component in a concentration from about 17.38 to about 21.68 moles per liter of the total volume of the solubility enhancing composition; a dilute sodium hydroxide solution having a concentration of about 5 percent to about 7.5 percent weight/weight of the total aqueous phase weight of the paper enhancing composition wherein the dilute sodium hydroxide solution has a concentration from about 20 percent to about 50 percent sodium hydroxide; at least one surfactant selected from the group consisting of non-ionic surfactant and anionic surfactant having a concentration from about 0.05 percent to about 0.15 percent weight/weight of the total aqueous phase weight of the paper enhancing composition; silver sulfate having a concentration from about 0.001 percent to about 1.5 percent weight/weight of the total weight of the paper enhancing composition; and at least one acid or at least one base to adjust the final pH of the paper enhancing composition in a range from about pH 2.5 to about pH 3.5.

The present invention further provides a method of increasing at least one of the group consisting of paper tensile, bond and burst strength of paper comprising the addition of at least one paper enhancing composition of the present invention to during or following the paper making process (e.g., a paper coating) compared to a paper making process not using such paper enhancing composition.

The present invention also provides a method of increasing at least one of paper tensile strength, bond strength and burst strength compared to paper prepared without the addition of at least one paper enhancing composition comprising the addition of at least one paper enhancing composition to a substrate slurry stage or to the wet-end stage of the paper making process.

Another aspect of the present invention provides a method for decreasing the interstitial pore size between and among paper fibers in a wet-end-paper making process compared to paper prepared without the addition of at least one paper enhancing composition comprising the addition of at least one paper enhancing composition to the substrate slurry stage or wet-end stage of the paper making process.

An additional aspect of the present invention provides a method for increasing paper density compared to paper prepared without the addition of at least one paper enhancing composition comprising the addition of at least one paper enhancing composition to the substrate slurry stage or wet-end stage of the paper making process.

A further aspect of the present invention provides for paper having antimicrobial properties comprising paper prepared using at least one paper enhancing composition during the paper making process or afterward (e.g., as a paper coating or as one aspect of a paper coating).

Also provided herein is a method of modifying the zeta potential of calcium carbonate when used in the paper making process comprising adding at least one aqueous carbonate enhancing composition to calcium carbonate or other fill material prior to the introduction of such calcium carbonate or other fill material to the paper making process as further described herein.

Another aspect of the present invention provides for enhanced paper comprising paper having applied to such paper at least one aqueous enhancing paper composition during any stage of the paper making process or afterward (e.g., as a paper coating or as one aspect of a paper coating).

Further provided herein are the following methods:

A method of enhancing paper comprising applying at least one aqueous paper enhancing composition during any stage of the paper making process or afterward (e.g., as a paper coating or as one aspect of a paper coating).

A method of increasing at least one of the group consisting of tensile strength, bond strength and burst strength in paper compared to the respective tensile strength, bond strength and burst strength of paper untreated with an aqueous paper enhancing composition comprising applying at least one aqueous paper enhancing composition during any stage of the paper making process or afterward (e.g., as a paper coating or as one aspect of a paper coating).

A method of increasing at least one of the group consisting of paper tensile strength, bond strength and burst strength of paper comprising applying at least one aqueous paper enhancing composition during any stage of paper production, typically the wet-end stage, compared to paper untreated with an aqueous paper enhancing composition without an increase in caliper pose.

Further provided is antimicrobial paper, having a multitude of uses, comprising paper prepared by the application of at least one aqueous paper enhancing composition of the present invention during any stage of paper production including, for example and without limitation, a paper coating stage.

Another aspect of the present invention provides for a paper coating comprising at least one aqueous paper enhancing composition.

An additional aspect provides for paper coated with at least one aqueous paper enhancing composition.

Another aspect of the present invention provides a method of increasing at least one of the group consisting of paper tensile strength, bond strength and burst strength of paper comprising the application of a coating to paper comprising at least one paper enhancing composition of the present invention.

An additional aspect of the present invention provides for a method of providing at least one of protection from fingerprints and other blemishes, help prevent metallic inks from tarnishing, and provide paper surfaces that can be written on with multiple media (including, without limitation, pencil, pen, ink jet printers, laser jet printers off-set printers and the like) comprising the application of a coating to paper comprising at least one paper enhancing composition of the present invention.

A further aspect of the present invention provides for a method of providing improvement of at least one of protection from fingerprints and other blemishes, help prevent

metallic inks from tarnishing, and provide paper surfaces that can be written on with multiple media (including, without limitation, pencil, pen, ink jet printers, laser jet printers off-set printers and the like) compared to paper coatings not including the application of at least one aqueous paper enhancing composition of the present invention comprising the application of a coating to paper comprising at least one paper enhancing composition of the present invention.

10 Accordingly, another aspect of the present invention provides for coated paper having antimicrobial activity comprising paper coated with at least one aqueous paper enhancing composition of the present invention.

An additional aspect of the present invention provides for 15 paper having antimicrobial properties comprising paper made with or coated with at least one aqueous paper enhancing composition of the present invention.

Another aspect of the present invention provides for a 20 method of preparing paper having antimicrobial activity comprising applying as a coating to paper at least one aqueous paper enhancing composition of the present invention to said paper.

Another aspect of the present invention provides a method 25 of extending the shelf-life of perishable foodstuff comprising placing such foodstuff in contact with paper made with and/or coated with at least one aqueous paper enhancing composition of the present invention. Such shelf-life can be extended for at least 24 hours compared to a paper product 30 that was untreated with a paper enhancing composition, providing substantial value to providers of such perishable foodstuff.

Further provided is a method for preparing paper for 35 medical and industrial protective uses comprising applying as a coating to paper at least one aqueous paper enhancing composition.

An additional aspect provides a method of preparing paper for use in masks for mammalian, particularly human, use comprising applying as a coating at least one aqueous paper enhancing composition.

An additional aspect of the present invention provides a 40 carbonate enhanced composition comprising at least one carbonate or other fill material and at least one carbonate enhancing composition.

A further aspect of the present providers a carbonate 45 enhancing composition which is the same as each paper enhancing composition as taught herein. These compositions differ in their uses wherein paper enhancing compositions are used as described herein whereas carbonate enhancing compositions are used to prepare enhanced carbonate compositions or for enhancing other fill materials, also as further described herein.

Another aspect of the present invention provides for a 50 carbonate enhancing composition consisting of: a solubility enhancing composition comprising an anionic component comprising sulfate ions, alone or in combination with bisulfate ions, having a concentration from about 8.00 moles per liter to about 13.00 moles per liter of the solubility enhancing composition volume, a cationic component comprising ammonium ions having a concentration from about 1.45 moles per liter to about 2.01 moles per liter of the solubility 55 enhancing composition volume, and a hydrogen ion component in a concentration from about 17.38 to about 21.68 moles per liter of the total volume of the solubility enhancing composition; a dilute sodium hydroxide solution having a concentration of about 5 percent to about 7.5 percent weight/weight of the total aqueous phase weight of the paper enhancing composition wherein the dilute sodium hydroxide

solution has a concentration from about 20 percent to about 50 percent sodium hydroxide; at least one surfactant selected from the group consisting of non-ionic surfactant and anionic surfactant having a concentration from about 0.05 percent to about 0.15 percent weight/weight of the total aqueous phase weight of the paper enhancing composition; silver sulfate having a concentration from about 0.001 percent to about 1.5 percent weight/weight of the total weight of the paper enhancing composition; and at least one acid or at least one base to adjust the final pH of the paper enhancing composition in a range from about pH 2.5 to about pH 3.5.

Other aspects of the present invention provide a variety of methods of using a carbonate enhanced composition of the present invention to a variety of intermediate and final products as further described herein below.

An additional aspect of the present invention provides a carbonate enhancing composition comprising an aqueous phase comprising a solubility enhancing aqueous composition wherein 1 part of a first solution is added to about 15 to about 20 parts of water to form a second solution; sodium hydroxide solution having a concentration of about 5% to about 7.5% weight/weight of the total aqueous phase weight of the composition; at least one surfactant selected from the group consisting of non-ionic surfactants and anionic surfactants having a concentration from about 0.05 percent to about 0.15 percent weight/weight of the total aqueous phase weight of the composition; and copper sulfate having a concentration from about 20 percent to about 26 percent weight/weight of the total aqueous phase weight of the composition; optionally comprising the addition of at least one acid or at least one base to adjust the final composition pH to a pH of about 2.5 to about 3.5.

Another aspect of the present invention provides a carbonate enhancing composition comprising an aqueous phase comprising a solubility enhancing aqueous composition wherein 1 part of a first solution is added to about 15 to about 20 parts of water to form a second solution and sodium hydroxide solution having a concentration of about 5% to about 7.5% weight/weight of the total aqueous phase weight of the composition; and copper sulfate having a concentration from about 20 percent to about 26 percent weight/weight of the total aqueous phase weight of the composition, optionally comprising the addition of at least one acid or at least one base to adjust the final composition pH to a pH of about 2.5 to about 3.5.

An additional aspect of the present invention provides an antimicrobial composition comprising at least one composition selected from the group consisting of at least one carbonate enhanced composition and at least one carbonate enhancing composition, wherein the carbonate enhancing composition is optionally aqueous or substantially aqueous.

A further aspect of the present invention provides a product requiring at least one carbonate as an element in the manufacture thereof comprising at least, in part, one carbonate enhanced composition used in the manufacture of such product.

An additional aspect of the present invention provides an antimicrobial composition comprising at least one carbonate enhanced composition.

To prepare a carbonate enhanced compositions for use in the paper making process, at least 1.5 pounds weight/weight of at least one carbonate enhancing composition of the present disclosure is added, typically as a spray designed to provide thorough coverage of the fill material, generally calcium carbonate particles, to each ton of one or more selected fill material, typically one or more calcium carbon-

ate products. Up to about twelve pounds or greater of carbonate enhancing composition per ton of calcium carbonate weight/weight can be used to prepare a carbonate enhanced compositions for use in paper. More particularly, 5 any whole or fractional number of the enumerated range of pounds of carbonate enhancing composition per ton of calcium carbonate is used to prepare a carbonate enhanced composition for use in paper. The use of the term "ton" as used herein refers to the U.S. ton. Slight proportionate 10 adjustments of the amount of addition of a carbonate enhancing composition per ton of calcium carbonate or other selected fill material may have to be made if tonnage is determined as metric tons or a British (long) ton. Any calcium carbonate product(s) used as filler for making paper can be used to prepare carbonate enhanced compositions of 15 the present invention. Selection of the amount of carbonate enhancing composition added to calcium carbonate to prepare carbonate enhanced compositions for use in paper may be judicially selected by the manufacturer of either the 20 calcium carbonate and/or the paper producer based on the type of paper (including paperboard) and/or the use of the paper product(s). Furthermore, the use of carbonate enhanced compositions of the present invention should not be restricted by the use of other additives typically used in 25 the paper manufacturing process.

To impart the antimicrobial properties in paper referenced herein, typically, at least 5 pounds of carbonate enhancing composition is used for each ton of calcium carbonate to form carbonate enhanced compositions although less may be 30 adequate for certain paper uses. More particularly, the amount of calcium enhancing composition added to calcium carbonate for such antimicrobial uses in paper is, for example, 5 pounds, 6 pounds, 7 pounds, 8 pounds, 9 pounds, 10 pounds, 11 pounds and greater than 12 pounds, or any 35 whole or fractional number within the stated range, per ton of calcium carbonate.

For paper pulp, at least one carbonate enhanced composition, typically using calcium carbonate, can also be used as 40 a causticizing agent in the pulp sulfate process, to prepare calcium bisulfate in the pulp sulfite process, used with chlorine in the bleaching process, in the treatment of pulp and paper mill waste treatment, a filtration conditioner, a neutralizing agent and/or to recover alcohol, calcium lignosulfonate and yeast.

The present invention further provides a paper enhancing composition comprising water, at least one solubility enhancing aqueous composition, sodium hydroxide, copper sulfate and/or silver sulfate and optionally, at least one surfactant selected from the group consisting of non-ionic surfactants and/or anionic surfactants.

An additional aspect of the present invention provides an aqueous or, substantially aqueous, paper enhancing composition (aqueous notwithstanding the potential for copper sulfate and/or silver sulfate to not have completely dissolved 55 in the paper enhancing composition) comprising an aqueous phase comprising a solubility enhancing aqueous composition wherein 1 part of a first solution is added to about 15 to about 20 parts of water, frequently deionized water, to form a second solution; sodium hydroxide solution having a 60 concentration of about 5% to about 7.5% weight/weight of the total aqueous phase weight of the paper enhancing composition; at least one surfactant selected from the group consisting of non-ionic surfactants and anionic surfactants having a concentration from about 0.05 percent to about 0.15 percent weight/weight of the total aqueous phase weight of the paper enhancing composition; and copper sulfate having a concentration from about 20 percent to

about 26 percent weight/weight of the total aqueous phase weight of the paper enhancing composition. The use of such surfactant in the present composition is optional. As used herein, the term "aqueous paper enhancing composition" also includes any such composition that is substantially aqueous as indicated above.

The immediately above-referenced composition can replace copper sulfate with silver sulfate wherein the concentration of silver sulfate is from about 0.001 percent to about 1.5 percent weight/weight of the total aqueous phase weight of the paper enhancing composition.

A further aspect of the present invention further comprises the addition of an acid or base to adjust the pH to a pH from about 2.5 to about 3.5 to the preceding paper enhancing compositions.

There are multiple potential uses of such paper enhancing compositions throughout paper making and paper finishing processes. For example, paper enhancing compositions of the present invention can be added directly to the wet-end stage of paper production for use as, for example, a paper coagulator and/or to provide microbial control.

As a coagulator, the addition of at least one paper enhancing composition to the wet-end of paper production can increase the tensile strength, bond strength and/or burst strength of paper through multiple actions. Without being held to a particular theory, it is believed that the addition of at least one paper enhancing composition of the present invention creates an environment wherein the fiber(s) used in paper making, with or without the presence of calcium carbonate or other fill material, enhances the attraction of the fibers, narrowing the interstitial spaces between and among fibers creating smaller pores while increasing the tensile, bond and/or burst strength of the resulting paper. The purpose for using such paper enhancing compositions in this context is to impart additional paper strength compared to paper produced without the use of such paper enhancing compositions without affecting paper caliper or pose or, alternatively, increased amount of such paper enhancing compositions can be used to increase the density of the resulting paper for a variety of uses including, for example and without limitation, preparation of paper, frequently in the form of masks, used for industrial and/or medical use wherein the passage of pollutions and/or microorganisms are retarded or prevented.

It is believed that the addition of at least one paper enhancing composition of the present invention modifies the zeta potential of the calcium carbonate, when calcium carbonate is used as a filler material, modifying the charge of the calcium carbonate and potentially providing stronger bond/interaction between the fiber and calcium carbonate filler. Such modification of the zeta potential frequently provides an increase in the zeta potential when a paper enhancing composition is added before, during or after the wet end is formed while the paper enhancing composition is typically applied to the wet end of the paper making process.

To use the aqueous paper enhancing compositions and impart the benefits of the use thereof including, for example and without limitation, paper coagulation and antimicrobial activity, at least one aqueous paper enhancing compositions is added to the wet-end of a paper making process at a concentration of about at least 1,500 ppm weight/weight of the total weight of the wet-end mixture to which the paper enhancing composition(s) is/are added. More specific amounts of paper enhancing compositions (aqueous or substantially aqueous) are added, typically, to the wet-end processes at concentrations of about 1,500 ppm, about 2,500 ppm, about 3,500 ppm, about 4,500 ppm, about 5,500 ppm,

about 6,500 ppm or greater than about 7,000 ppm weight/weight of the total weight of the wet-end mixture to which the paper enhancing composition(s) is/are added. Moreover, any whole or fractional number of ppm of the stated range of paper enhancing composition may be added to the wet-end mixture to which the paper enhancing composition(s) is/are added. Selection of the amount of paper enhancing composition added to the wet-end mixture to which the paper enhancing composition(s) is/are added may be judicially selected by the paper producer based on the type of paper and/or the intended use of paper product(s). Furthermore, the use of paper enhanced compositions of the present invention should not be restricted by the use of other additives typically used in the paper manufacturing process.

To impart the antimicrobial properties in paper referenced herein, typically, at least 2,500 ppm of the at least one paper enhancing composition is added or applied per ton of the wet-end mixture to which the paper enhancing composition(s) is/are added. More particularly, the amount of paper enhancing composition added or applied to the wet-end mixture to which the paper enhancing composition(s) is/are added for such antimicrobial uses in paper is, for example, about 2,500 ppm, about 3,500 ppm, about 4,500 ppm and greater than about 5,000 ppm, or any whole or fractional number thereof, per ton of wet-end mixture.

Notwithstanding the teachings for wet-end use of carbonate enhancing compositions and paper enhancing compositions of the present invention, a paper producer may not wish to enhance all of the paper produced from pulp or another fiber to the final product. It is beneficial for a paper producers to select which paper products may be treated to impart additional qualities to the final paper products. Such additional qualities can be imparted into or onto paper via the application of a paper enhancing composition of the present invention via application of such composition onto paper before, during or after the wet press aspect of paper production. Typically, after the wet-end step of paper production is completed, the mix of fiber, filler and any additional components is fed through a series of high pressure rollers for the purpose of squeezing out a substantial amount of water from the wet-end prior to the paper entering dryer and calendar sections. High pressure roller systems can be fitted with spray nozzles before, during or after the wet press section. It is throughout this wet press section of paper processing that one or more paper enhancing compositions of the present invention is/are sprayed onto the paper.

Application, typically as a spray, of at least one paper enhancing composition onto paper entering, during or following the wet press section of the paper making process can impart the same and additional benefits and attributes to paper as with the use of adding at least one carbonate enhanced composition and/or at least one paper enhancing composition of the present invention during the wet-end process as described herein. As such, application of at least one aqueous paper enhancing composition of the present invention can provide increased tensile, bond strength and/or burst strength to the respective paper, modify the zeta potential of calcium carbonate or at least one enhanced carbonate composition of the present invention used in the paper making process applied when the paper carries a substantial amount of water/moisture (e.g., the earlier to mid stages of the wet press process), improved hydrophobic sizing, opacity, and print characteristics, while potentially not affecting paper caliper or caliper pose unless otherwise intended. When desired, however, the density of paper can be increased by reducing pore spaces between and among the fiber and/or fill particles via the application of at least

one aqueous paper enhancing composition of the present invention during the wet press stage of production. The resulting paper can be used for medical and industrial applications, providing improved safety compared to products prepared without the benefit of the aqueous paper enhancing compositions. As further referenced herein, the aqueous paper enhancing compositions of the present invention also provide antimicrobial activity into and potentially throughout the paper onto which the present composition is applied during the wet press process of paper making. Collectively, the attributes presented in this paragraph represents, for the purposed herein, as "enhanced paper", and the process of preparing enhanced paper as "enhancing paper".

To use the aqueous paper enhancing compositions and impart the benefits of the use thereof including, for example and without limitation, paper strengthening and antimicrobial activity, at least one aqueous paper enhancing compositions is applied, typically as a spray, before, during or after the wet press stage of a paper making at a concentration of about at least 1,500 ppm weight/weight of such composition to each ton of wet weight matter entering the wet press stage. More specifically, amounts of paper enhancing compositions are applied as a spray during the wet press stage of paper making at concentrations of about 1,500 ppm, about 2,500 ppm, about 3,500 ppm, about 4,500 ppm, about 5,500 ppm, about 6,500 ppm or greater than about 7,000 ppm (as high as 20 ppm) to each ton of wet weight matter entering the wet press stage of paper making. Generally, concentrations of paper enhancing compositions can be reduced at later stages of the wet press stage if the spray containing paper enhancing compositions is applied after a substantial amount of moisture is removed. However, if the spray containing paper enhancing compositions of the present invention is applied once the paper is substantially dry but prior to entering the drying process, it is suggested to use the spray concentrations set forth below for paper coatings. However, slightly higher concentrations should be used based on the amount of residual moisture prior to such drying stage. Moreover, any whole or fractional number of ppm, within the stated concentration range, of paper enhancing composition may be applied during the wet press stage. Selection of the amount of paper enhancing composition applied during the wet press stage may be judicially selected by the paper producer based on the type of paper (including paper board) and/or the use of the paper product(s). Furthermore, the use of paper enhanced compositions of the present invention should not be restricted by the use of other additives typically used in the paper manufacturing process.

To impart the antimicrobial properties in paper referenced herein, typically, at least 2,500 ppm weight/weight of the at least one paper enhancing composition is applied for each ton of wet weight matter entering the wet press stage. More particularly, the amount of paper enhancing composition applied during the wet press stage for such antimicrobial uses in paper is, for example, about 2,500 ppm, about 3,500 ppm, about 4,500 ppm and greater than about 5,000 ppm, or any whole or fractional number thereof, per ton of wet weight matter entering the wet press stage of paper production. The amount of paper enhancing composition used can be adjusted pursuant to the recommendations set forth in the immediately preceding paragraph.

Alternatively, at least one of the aqueous paper enhancing compositions of the present invention can be applied to paper as an additive to surface sizing, wherever surface sizing is applied throughout the paper and or paper printing processes. The concentrations of at least one paper enhanc-

ing composition of the present invention when applied with sizing are the same concentrations taught herein below for the concentrations used for paper coatings. The only difference is that the concentrations are based on the total volume of sizing being surface applied to paper rather than the total volume of paper coating(s) being applied. As such, a minimum recommended concentration of at least one paper enhancing composition of the present invention to be applied with surface sizing is at least about 1,500 ppm of the total sizing volume being surface applied for general use and benefit; and at least about 2,500 ppm of such paper enhancing composition when antimicrobial activity is desired.

Originally, it was believed that concentration of silver sulfate in the various compositions herein containing silver sulfate should be between about 20 percent to about 26 percent weight/weight of the total aqueous phase weight of a respective enumerated composition. It has since been discovered that the beneficial effects of the present compositions may be derived by the reduction or elimination of copper sulfate and/or silver sulfate. The removal or non-inclusion of copper sulfate and/or silver sulfate is not expected to substantially affect the use of such mixtures or compositions as set forth herein in the preparation of paper and/or paper products. Otherwise, a reduced concentration of silver sulfate may be beneficial to the preparations of the mixtures and compositions taught herein, and would be required if the intended use of an intermediate or final paper product is to have antimicrobial activity embedded therein. Further, it was discovered that the present mixtures and compositions using silver sulfate at concentrations greater than about 1.5 percent weight/weight of the weight of the respective composition, such as, for example, the paper enhancing and/or carbonate enhancing compositions, turned paper surfaces the color black, or overwhelmed any desired coloring other than black, resulting in a commercially unacceptable compositions. The resulting black color was sufficiently intense and steadfast that the black color could not typically be removed with via traditional methods and could not be overcome by using additional coloring when the final color of a desired final product was desired to be other than black. The inventors dedicated substantial research and development time and effort to develop a composition containing silver sulfate that maintained substantial and required antimicrobial activity while not turning targeted surfaces black. As such, the concentration of silver sulfate in any of the mixtures and compositions taught herein can range from about 0.001 percent to about 1.5 percent weight/weight of the weight of the respective composition as further described in additional detail herein. For the sake of clarity, the concentration of silver sulfate can be any whole or fractional number withing the stated range.

The concentration of silver sulfate used in paper enhancing and carbonate enhancing compositions can vary although the amount of silver sulfate used in these compositions typically is not greater than about 1.5 percent weight/weight of the weight of the respective composition. Such compositions can be applied or added to a fill material, typically calcium carbonate, in addition to starch used in the paper making process and or the wet end process. Generally, silver sulfate, as referenced above, is used at a concentration of about 0.001 percent to about 1.5 percent weight/weight of the weight of the respective composition. For application to and blending with a fill material, typically calcium carbonate to form an enhanced carbonate composition, the silver sulfate concentration can be narrowed to about 0.05 percent to about 0.50 percent weight/weight of the weight of the respective composition.

For each use of an aqueous paper enhancing compositions of the present invention, application during the paper making process as described above or when used as paper coatings as described below, such compositions can be applied individually or in combination with other additives and/or coating material as such materials are used in the paper making/processing arts.

Applications of at least one aqueous paper enhancing composition of the present invention can also be applied directly to finished paper at any time following the dryer section of the paper making process. In other words, such application can be made from the calendar section of paper making through and following printing thorough a printing press or other printing method; or, alternatively, to prepared paper products or directly to final paper products.

In addition to coatings being applied by the paper manufacturer, liquid coatings are frequently applied in-line by the printer as part of the printing process or off-line after the project leaves the press. Although the paper enhancing compositions of the present invention can be applied with any liquid coating, the present paper enhancing compositions are typically applied with commonly used or specialty aqueous coatings that are usually flooded across the entire sheet. Different coatings are available in different finishes, tints, textures and thicknesses, which may be used to adjust the level of protection or achieve different visual effects. Areas that are heavily covered with black ink or other dark colors often receive a protective coating to guard against fingerprints, which stand out against a dark background. Coatings are also used on magazine and report covers and on other publications that are subject to rough or frequent handling. Moreover, communicable diseases caused by microorganisms, particularly, without limitation bacteria, including MRSA, and viruses such as noroviruses and coronaviruses, each of which, along with other pathogens, have the ability to remain viable and transmissible on surfaces, including paper, for a period of time. Accordingly, it is beneficial to have additional materials that can be added to liquid paper coatings to impart attributes such as additional tensile strength, bond strength and/or burst strength to coated paper. Additionally, it is beneficial to provide antimicrobial attributes to the surface of paper through coatings. Each of these attributes can be added to paper via the application of at least one paper enhancing composition of the present invention as a component in other liquid, commonly aqueous, paper coatings or at a particular concentration to other acceptable paper coating media, including water. Coatings including at least one paper enhancing composition of the present invention can be applied via any method used in the paper coating industry including, for example and without limitation, flood coating, blade coating, premetered film presses and roll metering. Each type of coating has particular uses, benefits and drawbacks. As such, the applier of such coatings can select the best coating and type of application for each such coating application. Accordingly, the application of at least one paper enhancing composition of the present invention should not be limited by the type of paper coating or method of application.

As such, another aspect of the present invention provides for a paper coating comprising at least one aqueous paper enhancing composition.

An additional aspect provides for paper coated with at least one aqueous paper enhancing composition.

Paper, including the printing on paper, can also be enhanced and protected by a variety of well-known liquid additives. The present aqueous paper enhancing compositions of the present invention, when applied as paper coat-

ings alone or in combination with other paper coating materials including, for example and without limitation, varnish and ultra violet coatings, can also provide, for example and without limitation: protection from fingerprints and other blemishes, help prevent metallic inks from tarnishing, and provide surfaces that can be written on with pencil, pen, ink jet printers, laser jet printers, off-set printers and the like. Although the present aqueous paper enhancing compositions can be applied to paper, in general, it may be best to use 80 #text weight or heavier paper stocks to keep the paper from becoming curled or wrinkled, particularly when using a flood coating method.

Because of the antimicrobial activity of the present paper enhancing compositions of the present invention, such compositions can be used as coatings to paper to provide such antimicrobial activity. Paper coated with such compositions have almost unlimited uses including, for example and without limitation, construction of masks used for industrial pollutants and/or medical masks used by any individuals including medical and first-responder personnel, paper used for wrapping food products including produce and/or fish and/or meat products, paper used as or in diapers, in produce and/or fish and/or meat products (for example, the absorbent paper underlining packaged poultry products), packaging, generally, blotters used by children and/or adults, facial tissues, sanitary napkins, liners for fruit, or any of a plethora of other paper uses where the inhibition of microorganism is desired and/or required.

Accordingly, another aspect of the present invention provides for coated paper having antimicrobial activity comprising paper coated with at least one aqueous paper enhancing composition of the present invention.

An additional aspect of the present invention provides for paper having antimicrobial properties comprising paper coated with at least one aqueous paper enhancing composition of the present invention.

Another aspect of the present invention provides for a method of preparing paper having antimicrobial activity comprising applying as a coating to paper at least one aqueous paper enhancing composition of the present invention to said paper.

Further provided is antimicrobial paper, having a multitude of uses, comprising paper prepared by the application of a coating of at least one aqueous paper enhancing composition of the present invention during the wet press stage or other stage of paper production.

Because of the antimicrobial activity of paper coated with at least one such aqueous paper enhancing composition, such coated paper can protect and potentially prolong the shelf-life of produce, meats and other perishable foodstuff (collectively, "foodstuff"). As such, another aspect of the present invention provides a method of extending the shelf-life of perishable foodstuff comprising placing such foodstuff in contact, in whole or in part, with paper coated with or made with at least one aqueous paper enhancing composition of the present invention. Such shelf-life can be extended for at least 24 hours, providing substantial value to providers of such perishable foodstuff.

Another aspect provides a method for preparing paper for medical and industrial protective uses comprising applying as a coating to paper at least one aqueous paper enhancing composition during.

An additional aspect provides a method of preparing paper for use in masks for mammalian, particularly human, use comprising applying as a coating at least one aqueous paper enhancing composition.

Aqueous paper enhancing compositions of the present invention are applied to paper as coatings, either as a single coating in a liquid-based solution, frequently water, or as at least one component with other surface-applied paper coating materials at a concentration of at least about 1,500 ppm volume/volume of the total amount of liquid-based solution or coating being applied. More specifically, amounts of paper enhancing compositions are applied as a spray coating at concentrations of about 1,500 ppm, about 2,500 ppm, about 3,500 ppm, about 4,500 ppm, about 5,500 ppm, about 6,500 ppm or greater than about 7,000 ppm of the total amount of liquid-based solution or coating being applied. Moreover, any whole or fractional number of ppm of paper enhancing composition, within the given concentration range, may be applied during the coating process. Selection of the amount of paper enhancing composition applied during the coating process stage may be judicially selected by the paper producer, printer, or desire of the end user based on the type of paper (including paper board) and/or the use of the paper product(s).

To impart the antimicrobial properties in paper referenced herein, typically, aqueous paper enhancing compositions of the present invention are applied to paper as coatings, either as a single coating in a liquid-based solution, frequently water, or as at least one component with other surface-applied paper coating materials at a concentration of at least about 2,500 ppm of the total amount of liquid-based solution or coating being applied. More specifically, to provide antimicrobial properties to paper coatings, amounts of paper enhancing compositions are applied as a spray coating at concentrations of about 2,500 ppm, about 3,500 ppm, about 4,500 ppm, about 5,500 ppm, about 6,500 ppm or greater than about 7,000 ppm of the total amount of liquid-based solution or coating being applied to the paper. Moreover, any whole or fractional number of ppm of paper enhancing composition within the given concentration range, may be applied during the coating process. Selection of the amount of paper enhancing composition applied during the coating process stage may be judicially selected by the paper producer, printer, or desire of the end user based on the type of paper (including paper board) and/or the use of the paper product(s).

For each of the claims set forth herein below, such claims can be alternatively drafted using "consisting of" and "consisting essentially of" claim language.

One element of the present paper enhancing compositions and carbonate enhancing compositions of the present invention provides a solubility enhancing aqueous composition comprising a first solution comprising an anionic component consisting essentially of sulfate ions, alone or in combination with bisulfate ions, having a concentration from about 8.00 moles per liter to about 13.00 moles per liter of the first solution volume, and a cationic component consisting essentially of ammonium ions having a concentration from about 1.45 moles per liter to about 2.01 moles per liter of the first solution volume, combined with a volume of water at least equal to the volume of the first solution forming a second solution. The solubility enhancing composition can also be prepared without the addition of water by determining the final desired volume of water prior to preparation and ensuring the preparation results in the composition having the stated ion concentration ranges for the anionic, cationic and hydrogen elements within such solubility enhancing composition. Generally, the first solution of this composition will also comprise hydrogen ions in a concentration from about 17.38 to about 21.68 moles per liter of the total volume of the first solution.

An alternative element of the present paper enhancing composition provides a solubility enhancing aqueous composition comprising a first solution comprising an anionic component comprising sulfate ions, alone or in combination with bisulfate ions, having a concentration from about 8.00 moles per liter to about 13.00 moles per liter of the first solution volume, and a cationic component comprising ammonium ions having a concentration from about 1.45 moles per liter to about 2.01 moles per liter of the first solution volume, combined with a volume of water at least equal to the volume of the first solution forming a second solution. Generally, the first solution of this composition will also comprise hydrogen ions in a concentration from about 17.38 to about 21.68 moles per liter of the total volume of the first solution, but a final solubility enhancing composition can be prepared by the ordinarily skilled artisan to have this same range of hydrogen ion concentration.

It is the intent of the present disclosure to permit the skilled artisan to prepare a solubility enhancing aqueous composition element using a range of water in a ratio to the concentrations of ammonium sulfate and sulfuric acid for each preparation, with the resultant sulfate anions and ammonium cations, and the amount of water to be determined by such artisan, each within the parameters taught herein.

For the sake of clarity, three solutions may be formed in preparing the second solution which comprise solubility enhancing aqueous compositions: 1) ammonium sulfate stock solution; 2) a first solution comprising the ammonium sulfate stock solution in sulfuric acid; and 3) second solution comprising solubility enhancing aqueous compositions. Unless context otherwise dictates, general references to the use of a first solution and a second solution refers to the preparation of the referenced solubility enhancing aqueous compositions used in the preparation of paper enhancing agent compositions of the present invention.

To prepare the first solution of a composition of the present disclosure, one needs to first prepare an ammonium sulfate stock solution. For example and without limitation, an ammonium sulfate stock solution is prepared to contain 20%, 24%, 30%, 40%, 50% or 60% of ammonium sulfate in water, typically, without restriction, deionized water. For the sake of clarity, the percent concentration of ammonium sulfate can be any whole number or fraction thereof in a range from about 20% to about 60%. The molar concentration of the stock solution varies by the ammonium sulfate concentration in a known volume of water.

By means of exemplification, the following calculations are used to determine the amount of ammonium sulfate and sulfuric acid to add to form a first solution.

#### Ammonium Sulfate:

Ammonium sulfate equals 132.14 grams per mole. Using, for example, a 24% ammonium sulfate solution, such solution would have 240 grams of ammonium sulfate per 1 L of water. Because the ratio of ammonium sulfate to sulfuric acid in this exemplification is about 48% ammonium sulfate to about 52% sulfuric acid, the first solution would contain 115.20 grams of ammonium sulfate, equaling 0.872 moles per liter. As such, one mole of ammonium sulfate provides 2 moles of ammonium and 1 mole of sulfate. Accordingly, 0.872 moles of ammonium sulfate provides to the ammonium sulfate stock solution 1.744 moles of ammonium and 0.872 moles of sulfate required per liter of reaction in forming the first solution.

## Sulfuric Acid (Concentrated):

Sulfuric acid equals 98.079 g/mole as concentrated (95% to 98%) reagent grade sulfuric acid. Sulfuric acid exists as a liquid and has a density of 1.840 g/mL. For this example, sulfuric acid comprises 52% of a first solution of 1 liter. As such, 520 mL (0.52 L) of sulfuric acid is added to the ammonium sulfate stock solution. 520 mL times 1.840 g/mL equals 956.8 grams. 956.8 grams divided by 98.079 grams per mole provides the target concentration of 9.755 moles of sulfuric acid per liter of preparation. 9.755 moles of sulfuric acid provides 9.755 moles of sulfate anion and 2 moles of hydrogen resulting from each mole of acid, in this example, 19.51 moles of hydrogen per liter of said first solution.

## Reaction Unit:

Using the values set forth above, in this instance, there are about 0.872 moles of ammonium sulfate to about 9.755 moles of sulfuric acid providing:

about 0.872 moles of ammonium sulfate provides about 0.872 moles of sulfate and about 1.744 moles of ammonium required per reaction unit liter; and about 9.755 moles per liter of sulfuric acid provides about 9.755 moles of sulfate anion and about 19.51 moles of hydrogen per liter of reaction unit.

Using this example, each reaction unit, forming a first solution, would contain:

about 0.972 moles of sulfate (from ammonium sulfate) plus about 9.755 moles of sulfate from ammonium sulfate equaling about 10.627 moles of sulfate anion per liter comprising sulfate anions alone, bisulfate anions alone or, typically, a mixture of sulfate and bisulfate anions;

about 1.744 moles of ammonium per liter; and about 19.51 moles of hydrogen per liter.

Generally, solubility enhancing compositions are free or substantially free of solids. Use of the solubility enhancing aqueous compositions may form solids when combined with other chemical or other materials when using such solubility enhancing aqueous compositions for its intended purpose: enhancing solubility of such chemical compounds or other materials.

Generally, water is at least fifty percent of a solubility enhancing aqueous compositions. Moreover, water can comprise from at least fifty percent up to ninety-nine percent of the second solution or final composition. However, the lower concentrations of water, as taught herein, are typically more useful for further use of the present compositions used for solubility enhancement or as used in the paper enhancing and/or carbonate enhancing compositions of the present invention. Accordingly, the amount of water used to form a second solution is at least 50% of the volume of the first solution or at least 50% of the mass of the final solubility enhancing composition. Alternatively, the mass of the sum of the ammonium ion concentration plus sulfate ion concentration in a first solution can also serve as the basis of the amount of water to be added to form a second solution wherein the amount of water added, by mass, to form a second solution equals at least 50% of the sum of the mass of ammonium ions plus sulfate ions. Another means by which to represent the amount of water added to the first solution is that the amount of water used to form a second solution is at least equal to the volume of the first solution or at least equal to the mass of the first solution. Alternatively, the mass of the sum of the ammonium ions plus sulfate ions in a first solution can also serve as the basis of the amount of water to be added to form a second solution wherein the amount of total water, including the water used

to solubilize the ammonium sulfate and added water, is at least equal to the sum of the mass of ammonium ions plus sulfate ions. As noted herein, a preparer of a solubility enhancing compositions can precalculate, using any of the referenced methods, to determine the total amount of water required relative to the amount of sulfuric acid and ammonium sulfate used to create a solubility enhancing composition having the respective cationic, anionic and hydrogen molar ion concentrations as set forth herein.

The amount of water used to prepare the second solution, representing solubility enhancing aqueous compositions, can be calculated in volume/volume (total volume of the first solution plus at least the same volume of water). Alternatively, the ratio of reactants to water (mass/mass) may be used. Using the values for ammonium sulfate and sulfuric acid from the above example, 115.20 grams of ammonium sulfate and 956.8 grams of sulfuric acid were used providing a sum of 1072 grams of reactants. Accordingly, for water to equal at least fifty percent of the final composition, at least 1072 grams of water are added to the first solution to form the second solution, a solubility enhancing aqueous composition. Alternatively, as referenced above, the amount of water used to form a second solution can be based on the total mass or volume of the first solution. Accordingly, any method taught herein can be used for calculating the amount of water required to form a second solution. As taught above, using the mass of the reactants to dictate the amount of water required to form a second solution is generally the minimum amount of water required to provide an aqueous solution and to impart the qualities of the compositions of the present invention as further delineated herein.

To achieve solubility enhancement, ranges of concentration of sulfate ions and ammonium ions in the solubility enhancing aqueous compositions are used while maintaining solubility enhancing aqueous compositions that are essentially free or are free of salt crystals or other solids from the reactants that form a solubility enhancing composition. Accordingly, a first solution or final solubility enhancing composition comprises an anionic component consisting essentially of sulfate ions, alone or in combination with bisulfate ions, having a concentration range from about 8.00 moles per liter to about 13.00 moles per liter of the respective volume. The first solution or final solubility enhancing composition also comprises a cationic component consisting essentially of ammonium ions having a concentration from about 1.45 moles per liter to about 2.01 moles per liter of the respective volume. Typically, when the lower values within the range for sulfate ions are selected for preparing a first solution, a lower value within the stated range for ammonium ions is selected and included in the preparation of the respective solution. Similarly, when higher values within the stated range for sulfate ions are selected for the preparation of a first solution or final solubility enhancing composition higher values of ammonium ions are selected for the preparation of a first solution. Although not imperative, typically, the sulfate ion concentration within the given range of from about 8.00 moles per liter to about 13.00 moles per liter of first solution volume or final solubility enhanced composition is proportionally commensurate with the range of ammonium ion concentration within the given the given range of from about 1.45 moles per liter to about 2.01 moles per liter of first solution volume or final solubility enhancing composition.

In another embodiment of the solubility enhancing aqueous compositions, a first solution comprises an anionic component comprising sulfate ions, alone or in combination with bisulfate ions, has a concentration range from about

8.00 moles per liter to about 13.00 moles per liter of the first solution volume. The first solution also comprises a cationic component comprising ammonium ions has a concentration from about 1.45 moles per liter to about 2.01 moles per liter of the first solution volume. Typically, when the lower values within the range for sulfate ions are selected for preparing a first solution, a lower value within the stated range for ammonium ions is selected and included in the preparation of the first solution. Similarly, when higher values within the stated range for sulfate ions are selected for the preparation of a first solution, higher values of ammonium ions are selected for the preparation of a first solution. Although not imperative, typically, the sulfate ion concentration within the given range of from about 8.00 moles per liter to about 13.00 moles per liter of first solution volume is proportionally commensurate with the range of ammonium ion concentration within the given the given range of from about 1.45 moles per liter to about 2.01 moles per liter of first solution volume. When prepared according to the solubility enhancing aqueous composition embodiments provided herein, the resulting hydrogen ion concentration will typically fall within the range from about 17.38 moles per liter to about 21.68 moles per liter of first solution volume or final solubility enhancing composition, as appropriate.

The process for preparing the solubility enhancing aqueous compositions can be carried out using traditional laboratory and safety equipment when using concentrated acid and water that could generate significant heat. Within these considerations, the selection of laboratory equipment is not critical to the formation of the solubility enhancing aqueous solutions or compositions. More particularly, the preparation of the first solution wherein the reactants ammonium sulfate stock solution is combined with sulfuric acid requires laboratory apparatuses that are approved for heat generation, splashing and, potentially, pressure relief. Accordingly, the first solution should be prepared in a laboratory vessel that is not sealed providing for pressure relief, rather than a potential hazardous situation with pressure build up in an unrated vessel. The ordinarily skilled artisan should be knowledgeable in the selection and use of such apparatuses.

For commercial-scale production of solubility enhancing aqueous compositions, the ordinarily skilled artisan will recognize that the reaction between the solubilized ammonium sulfate and sulfuric acid is typically exothermic. As such, a reaction vessel appropriate to safely contain and, typically, cool this reaction, is recommended. Commercial production of a first solution and a second solution, or a single, final solubility enhancing composition, can be accomplished using any of the teachings herein but on a larger scale than the laboratory scale teachings and examples disclosed herein. Moreover, such commercial production can be accomplished, without limitation, as taught herein or with equipment known to the ordinarily skilled artisan.

The order of adding the reactants to each other is not critical in the preparation of a first solution. Either the stock ammonium sulfate solution can be added to the sulfuric acid or, more typically, sulfuric acid is added to the stock ammonium sulfate stock solution to avoid the splattering typical of adding a solution containing water to acid. Typically, the heat generating reaction forming the first solution is permitted to run to conclusion, with the term "conclusion" having the meaning understood by the ordinarily skilled artisan, prior to adding the first solution to the required water or water to the first solution, without preference to the order of addition. For the sake of clarity, conclusion of the reaction between the ammonium sulfate stock solution and sulfuric

acid typically occurs when the reactants no longer produce an exothermic reaction and the temperature of the solution begins to decrease to ambient temperature.

Alternatively, the formation of a first solution is not required and the ammonium sulfate stock solution and sulfuric acid can be combined with the final desired volume of a solubility enhancing aqueous compositions. Accordingly, another aspect of the solubility enhancing aqueous compositions provides a solubility enhancing aqueous composition comprising an anionic component consisting essentially of sulfate anions having a concentration from about 8.00 moles per liter to about 13.00 moles per liter of about one-quarter of the final solubility enhancing aqueous composition volume and a cationic component consisting essentially of ammonium ions having a concentration from about 1.45 moles per liter to about 2.01 moles per liter of about one-quarter of the final solubility enhancing aqueous composition volume or less, and water comprising at least one-half of the final composition volume.

20 An alternate solubility enhancing aqueous composition comprises an anionic component comprising sulfate anions having a concentration from about 8.00 moles per liter to about 13.00 moles per liter about one-half of the final solubility enhancing aqueous compositions volume and a cationic component comprising ammonium ions having a concentration from about 1.45 moles per liter to about 2.01 moles per liter of about one half of the final solubility enhancing aqueous composition volume.

Another alternate solubility enhancing aqueous composition comprises an anionic component consisting essentially of sulfate anions having a concentration from about 8.00 moles per liter to about 13.00 moles per liter and a cationic component consisting essentially of ammonium ions having a concentration from about 1.45 moles per liter to about 2.01 moles per liter of the final solubility enhancing aqueous composition volume wherein said liter volume for calculation for the volume of water comprising the ammonium ions and sulfate anions comprises at least one percent of the total volume of the solubility enhancing aqueous composition.

40 A further alternate solubility enhancing aqueous composition comprises an anionic component consisting essentially of sulfate anions having a concentration from about 8.00 moles per liter to about 13.00 moles per liter of not more than about one-half of the final solubility enhancing aqueous composition volume and a cationic component consisting essentially of ammonium ions having a concentration from about 1.45 moles per liter to about 2.01 moles per liter of not more than about one-half the final solubility enhancing aqueous composition volume.

50 An additional alternate solubility enhancing aqueous composition comprises an anionic component comprising sulfate anions having a concentration from about 8.00 moles per liter to about 13.00 moles per liter of not more than about one-half of the final solubility enhancing aqueous composition volume and a cationic component comprising ammonium ions having a concentration from about 1.45 moles per liter to about 2.01 moles per liter of not more than about one-half the final solubility enhancing aqueous composition volume. Each of the above solubility enhancing compositions also provide hydrogen ion molar concentrations as set forth herein.

60 Although certain aspects of the solubility enhancing aqueous compositions allow for highly dilute concentrations for the ammonium cations and sulfate anions, specific concentrations of these ions can be calculated on a basis as if such combination were prepared on a per liter basis wherein the volume of such preparation comprises 1%, 10%, 20%, 30%,

40%, 48%, 50% or 60% of the total volume of the final solubility enhancing aqueous composition. For the sake of clarity, the volume of water can be any whole number or fraction thereof in a range from about 1% to about 60%. In addition, the volume of total water in each of the solubility enhancing aqueous compositions taught herein can be calculated by a variety of methods as taught herein and are not limited by any one teaching. As such, the amount of water used to form a second solution can be based on weight/weight (first solution weight to the weight of water added to form a second solution); mass/mass (first solution mass to the mass of water added to form a second solution; and mass/mass (the mass of the sum of ammonium ions and sulfate ions to the mass of total water in the second solution). Each of these methods can be used in a two-step process wherein a first solution is formed and water is added to form a second solution, or a one-step process where the elements of a second solution of the present invention are pre-calculated and added accordingly.

As referenced above, one aspect of the present invention provides an aqueous paper enhancing composition comprising an aqueous phase comprising: a solubility enhancing aqueous composition wherein 1 part of a first solution is added to about 15 to about 20 parts of water to form a second solution; sodium hydroxide solution having a concentration of about 5% to about 7.5% weight/weight of the total aqueous phase weight of the composition; at least one optional surfactant selected from the group consisting of non-ionic surfactant and anionic surfactant having a concentration from about 0.05 percent to about 0.15 percent weight/weight of the total aqueous phase weight of the composition; and copper sulfate having a concentration from about 20 percent to about 26 percent weight/weight of the total aqueous phase weight of the composition. A further aspect of the present invention further comprises the addition of an acid or base to adjust the pH to a pH from about 2.5 to about 3.5 to the immediately preceding composition.

An additional aspect of the present invention provides an aqueous paper enhancing composition (or a carbonate enhancing composition) comprising a solubility enhancing aqueous composition comprising an anionic component comprising sulfate ions, alone or in combination with bisulfate ions, having a concentration from about 8.00 moles per liter to about 13.00 moles per liter of the solubility enhancing composition volume, a cationic component comprising ammonium ions having a concentration from about 1.45 moles per liter to about 2.01 moles per liter of the solubility enhancing composition volume, and a hydrogen ions component in a concentration from about 17.38 to about 21.68 moles per liter of the total volume of the solubility enhancing composition solution; a dilute sodium hydroxide solution (about 20% to about 50% dilution) having a concentration of about 5 percent to about 7.5 percent weight/weight of the total aqueous phase weight of the paper enhancing composition; at least one optional surfactant selected from the group consisting of non-ionic surfactant and anionic surfactant having a concentration from about 0.05 percent to about 0.15 percent weight/weight of the total aqueous phase weight of the paper enhancing composition; and silver sulfate having a concentration from about 0.001 percent to about 1.5 percent weight/weight of the total aqueous phase weight of the paper enhancing composition. This present aspect of the invention can also be prepared without silver sulfate.

A further aspect of the present invention further comprises the addition of an acid or base to adjust the pH to a pH from

about 2.5 to about 3.5 to the immediately preceding paper enhancing compositions with or without silver sulfate.

The paper enhancing or carbonate enhancing compositions of the present invention can be prepared using the total volume of the solubility enhancing composition as the basis for adding the additional elements of a paper enhancing composition or each element of a paper enhancing composition can be prepared with a desired final volume in which a solubility enhancing composition comprises from about 12 percent to about 35 percent weight/weight of the weight of the paper enhancing composition, with each of the additional elements as set forth herein having a concentration as stated herein in such desired final volume.

For the preparation of the above-referenced aqueous paper enhancing composition, a 20 percent to 50 percent dilute sodium hydroxide solution is prepared using techniques well known to the skilled artisan. The range of sodium hydroxide concentration in the present aqueous paper enhancing compositions is based on varied concentrations of sodium hydroxide. When higher concentration sodium hydroxide solutions are used, one would typically use the lower concentration range of about 0.5% weight/weight of the total aqueous element weight of the composition. Conversely, when lower concentration sodium hydroxide solutions are used, one would typically use the higher concentration range of about 0.75% weight/weight of the total aqueous element weight of the composition. Total aqueous element weight composition means the sum weight of the aqueous components of the present composition including the solubility enhancing aqueous composition, sodium hydroxide solution and surfactant.

Various aqueous concentrations of non-ionic and anionic surfactants are commercially available, frequently found in concentrations of about 20% to about 80% in water. Such surfactants can also be prepared by diluting concentrated non-ionic surfactant and/or anionic surfactants in water to desired concentrations. Accordingly, such surfactants having a concentration of 20%, 30%, 40%, 50%, 60%, 70% and 80% are useful in the present composition. Generally, surfactant concentrations of at least 20% in water are useful. More particularly, a 50% concentration of an alkyl polyglucocides surfactant (e.g., Glucopon® 420 in water; available from multiple vendors including, for example, BASF Corp., Florham Park, New Jersey, USA) is useful as a nonionic surfactant in the present aqueous paper enhancing compositions. When higher concentration surfactant solutions are used, one would typically use the lower concentration range of about 0.05% weight/weight of the total aqueous weight of the composition. Conversely, when lower concentration surfactant solutions are used, one would typically use the higher concentration range of about 0.15% weight/weight of the total aqueous element weight of the composition.

Additionally, a solubility enhancing aqueous composition is prepared wherein 1 part of a first solution, as described above, is added to about 15 to about 20 parts of water to form a second solution.

For preparation of the aqueous paper enhancing composition of the present invention, to the solubility enhancing aqueous composition is added dilute sodium hydroxide (about 20% to about 50%) having a concentration of about 5% to about 7.5% weight/weight of the total aqueous element weight of the composition. The surfactant element of the present composition can be added to this aqueous solution or can optionally be added following the addition of the copper sulfate and/or silver sulfate element. However, the calculation for the concentration of the surfactant is based on the total aqueous element weight of the composi-

tion as if the copper sulfate and/or silver sulfate had not yet been added. The at least one surfactant is selected from the group consisting of non-ionic surfactant and anionic surfactant having a concentration from about 0.05 percent to about 0.15 percent weight/weight of the total aqueous element weight of the composition.

The copper sulfate element of the present paper enhancing or carbonate enhancing compositions is added to such compositions described above at a concentration from about 20 percent to about 26% weight/weight of the total aqueous element weight of the composition.

The silver sulfate element of the present paper enhancing or carbonate enhancing compositions is added to such compositions described above at a concentration from about 0.001 percent to about 1.5 weight/weight of the total aqueous element weight of the composition.

Once the present composition is prepared, the final pH should be adjusted to a pH of from about 2.5 to about 3.5 with a pH of about 3.0 being typically used. Any base or acid can be used to increase or decrease, respectively, the pH of such a composition. However, it is best to utilize acids and bases already used in the present compositions; dilute sodium hydroxide to increase the pH and sulfuric acid to decrease the pH. Alternatively, pH is controlled throughout the various steps of preparation of an aqueous paper enhancing composition of the present invention. For example, pH can be adjusted to the ranges set forth above following the addition of dilute sodium hydroxide to the previously prepared solubility enhancing aqueous composition, and then again following the addition of copper sulfate and/or silver sulfate and optionally, following the addition of copper sulfate and/or silver sulfate and the anionic and/or nonionic surfactant. As such, the pH is adjusted at least one time during preparation of an aqueous paper enhancing composition, typically following the addition of the copper sulfate and/or silver sulfate and/or surfactant.

The process for preparing the paper enhancing compositions or carbonate enhancing compositions, can be carried out using traditional laboratory and safety equipment when using concentrated acid and water that could generate significant heat. Within these considerations, the selection of laboratory equipment is not critical to the formation of the carbonate enhancing compositions and/or aqueous carbonate enhancing compositions. The ordinarily skilled artisan should be knowledgeable in the selection and use of such apparatuses.

For larger scale production batches of such carbonate enhancing compositions of the present invention and aqueous paper enhancing compositions, such compositions are prepared based on the percentages taught herein above of the elements required for preparation of such compositions. As a non-limiting example, such compositions can be prepared as follows: to produce 330 gallons of finished product, to an adequate-sized tank having circulation mixing, is about 2,116 pounds of 17 meghohm water, typically, distilled water, about 183 pounds of a solubility enhancing aqueous composition, with continued mixing, about 183 pounds of 50% sodium hydroxide that is slowly added to the prior mixture, with continued mixing, about 590 pounds copper sulfate, with continued mixing to maintain the copper sulfate in solution, and about 2 pounds of 50% Glucopon® 420 UP, with continued mixing for at least about one hour. It is beneficial to adjust the pH after addition of each subsequent element beginning with the addition of the solubility enhancing aqueous composition. pH should be adjusted to be in the range from about pH 2.5 to about pH 3.5 with a median of pH 3.0 being a reasonable target. Alternatively,

silver sulfate can replace or be added in addition to the copper sulfate using about 4.86 pounds of silver sulfate.

The intent and benefit of the present paper enhancing and carbonate enhancing compositions is to provide an aqueous solution that free or substantially free of solids.

Although specific embodiments have been described above, these embodiments are not intended to limit the scope of the present disclosure, even where only a single embodiment is described with respect to a particular feature. Examples of features provided in this disclosure are intended to be illustrative rather than restrictive unless stated otherwise. The present disclosure is intended to cover such alternatives, modifications and/or equivalents as would be apparent to a person skilled in the art having the benefit of this disclosure.

It is to be understood that the present compositions are limited only to the ranges and or limitation set forth herein and not to variations within such ranges. It is also to be understood that the terminology used herein is for the purpose of describing particular embodiments only, and is not intended to be limiting.

Further modifications and alternative embodiments of various aspects of the embodiments described in this disclosure will be apparent to the skilled artisan in view of the present disclosure. Elements and materials may be substituted for those illustrated and described herein, parts and processes may be reversed, and certain features of the embodiments may be utilized independently, all as would be apparent to one skilled in the art after having the benefit of the description. Changes may be made in the elements described herein without departing from the spirit and scope of the appended claims.

## EXAMPLES

### Example 1

Preparation of an ammonium sulfate stock solution for a solubility enhancing aqueous composition: Into a volumetrically calibrated common 250 mL beaker, 90 mL of deionized H<sub>2</sub>O was added. 20 grams of (NH<sub>4</sub>)<sub>2</sub>SO<sub>4</sub> was completely dissolved into the deionized water. The total volume was brought to 100 mL using additional deionized water. 20 grams (NH<sub>4</sub>)<sub>2</sub>SO<sub>4</sub> per 100 mL H<sub>2</sub>O is a 20% solution and is a 1.51 M solution.

### Example 2

50 Direct preparation of a second solution for the preparation of a solubility enhancing aqueous composition without the prior preparation of a first solution wherein the ratio of a first solution equivalent to water addition in this step is four parts water to one part first solution equivalent:

55 1.15 mL of 20% (NH<sub>4</sub>)<sub>2</sub>SO<sub>4</sub> was added to a common 10 mL polypropylene centrifuge tube  
8.0 mL deionized water added to tube  
0.850 mL of concentrated (95-98%) sulfuric acid (H<sub>2</sub>SO<sub>4</sub>) added to tube with sufficient force to mix

### Example 3

60 Direct preparation of a second solution for a solubility enhancing aqueous composition without the prior preparation of a first solution wherein the ratio of a first solution equivalent to water addition in this step is nine parts water to one part first solution equivalent:

35

0.576 mL of 20%  $(\text{NH}_4)_2\text{SO}_4$  was added to a common 10 mL polypropylene centrifuge tube  
 9.0 mL deionized water added to tube  
 0.424 mL of concentrated (95-98%) sulfuric acid ( $\text{H}_2\text{SO}_4$ ) added to tube with sufficient force to mix

## Example 4

Direct preparation of a second solution for a solubility enhancing aqueous composition without the prior preparation of a first solution wherein the ratio of a first solution equivalent to water addition in this step is nineteen parts water to one part first solution equivalent:

0.288 mL of 20%  $(\text{NH}_4)_2\text{SO}_4$  was added to a common 10 mL polypropylene centrifuge tube  
 9.5 mL deionized water added to tube  
 0.212 mL of concentrated (95-98%) sulfuric acid ( $\text{H}_2\text{SO}_4$ ) added to tube with sufficient force to mix

## Example 5

Preparation of solubility enhancing aqueous composition samples for liquid chromatography—mass spectrometry (LC-MS) analysis: Each of Examples 2, 3 and 4, following addition of the sulfuric acid:

the centrifugation tubes were briefly capped and vortexed to mix thoroughly  
 caps were loosened to vent. It was observed that the temperatures of the centrifugation tubes were greater than ambient temperature. Such temperature was not sufficient to melt the centrifugation tubes.  
 reactions were allowed to run for about 60 minutes after completion of the reaction time, 1 mL samples of the reacted solutions were filtered through a 0.44 micron Pall syringe filter and placed into labeled mass spectrometry vials  
 vials were loaded into a Thermo Q Exactive Plus MS system with a Vanquish LC front end

LC Settings:  
 0.25 mL/min  
 40% methanol/60% water/0.1% formic acid column temp 30° C.  
 Thermo Accucore AQ C18 polar end cap column (150 mm×3 mm)

Injection volumes of 20  $\mu\text{L}$   
 Low resolution parameters

Full MS-SIM  
 0-10 minutes  
 Positive polarity  
 Resolution: 70,000  
 AGC Target:  $3 \times 10^6$   
 Max IT: 200 ms  
 Scan Range: 50-700 m/z

High resolution parameters  
 Full MS/dd-M52  
 0-7 minutes  
 Positive polarity  
 Full MS: Resolution: 70,500  
 AGC Target:  $3 \times 10^6$   
 Max IT: 100 ms

Scan range: 50-700 m/z  
 dd-MS<sup>2</sup>: Resolution: 17,500  
 AGC target:  $2 \times 10^6$   
 Max IT: 50 ms

Scan range: 50-700 m/z  
 Minimum AGC Target:  $2 \times 10^3$

36

Example 6: Laboratory Preparations of First Solutions for Preparation of Solubility Enhancing Aqueous Compositions for Ion Chromatographic Quantification

5 A 24% solution of ammonium sulfate was created by adding 96 grams of ammonium sulfate to 400 grams deionized water. The solution was mixed to completely dissolve the ammonium sulfate.

10 Ten (10) identical 20 mL reactions were produced: 9.6 mL of the preceding 24% ammonium sulfate solution was added to individually labeled common 50 mL conical tubes by way of calibrated macropipette  
 15 10.4 mL of concentrated sulfuric acid (95-98% reagent grade) was added to each tube by way of calibrated micropipette with sufficient force to thoroughly mix  
 Tubes were allowed to stand loosely capped for an hour for reaction to run to completion.

## Example 7: Ion Chromatography (IC) Method

Samples from Example 6 were transferred to IC vials, diluted appropriately (1:2500) to bring the ionic concentrations into the range of testing equipment used, and ion chromatography was undertaken using the following parameters:

Ion Chromatography:  
 Dual Thermo Dionex Aquion  
 Anion Side:  
 Column: Dionex IonPac AS22 RFID 4×250 mm  
 Mobile phase: carbonate/bicarbonate buffet at 4.8/1.2 mM  
 Flow: 1.2 mL/min isocratic  
 Suppressor: Dionex ADRS 600 4 mm  
 Sup. Voltage: 33 mA  
 Standard: IC STD for sulfate, 50-500 ppm  
 Anion cell: 35° C.  
 Anion column: 30° C.  
 18 minute run time  
 Cation Side:  
 Column: Dionex IonPac CS16 RFIC 5×250 mm  
 Mobile phase: 30 mM MSA solution  
 Flow: 1 mL/min isocratic  
 Suppressor: Dionex CDRS 600 4 mm  
 Sup. voltage: 89 mA  
 Standard: IC STD for ammonium 20-100 ppm  
 Cation cell: 40° C.  
 Cation column: 35° C.  
 18 minute run time  
 All 25  $\mu\text{L}$  injections

## Example 8. Ion Chromatography Results

Using the sample preparations set forth in Example 6 and the ion chromatography methods set forth in Example 7, the following results (10 samples; 2 replicates) were obtained:

|    | Sulfate mol/L           | Ammonium mol/L         |
|----|-------------------------|------------------------|
| 60 | 9.1904799<br>8.00-13.00 | 1.6264427<br>1.45-2.01 |

## Example 9: Commercial-Scale Production of a Solubility Enhancing Composition First Solution

65 Into a 500-gallon polyethylene conical-bottom tank was added 160.5 pounds (about 19.2 gallons) of deionized water.

37

Upon addition of the water, a magnetic-driven shearing pump with an impeller was engaged, circulating the water in the tank. To the water was slowly added 50.7 pounds of pre-weighed ammonium sulfate (GAC Chemical Corp., Searsport Maine, U.S.A.) to enable solubilization of the ammonium sulfate preparing a 31.6% ammonium sulfate solution. The recirculating pump was allowed to run for about 20 minutes for this batch size. Complete solubilization of the ammonium sulfate was visually confirmed by decanting about 250 mL of solution into a PET bottle that was allowed to stand undisturbed for about 15 minutes, confirming complete solubilization.

A 50-gallon Dietrich (Corpus Christi, Texas, U.S.A.) closed-loop, stainless steel-jacketed, glass-lined reactor was pre-cooled using a CTS T-230 cooling tower (Cooling Tower Systems, Macon, Georgia U.S.A.) circulating a mixture of municipal water and sufficient sodium hypochlorite to maintain a pH from about 7.5 to about 7.8. To this reactor was added 400.6 pounds (about 26.1 gallons) of 98% sulfuric acid (Brenntag; Henderson, Kentucky U.S.A.) while a shaft-driven paddle mixer was engaged at 1700 rpm. To the sulfuric acid was rapidly added the ammonium sulfate solution and was mixed for about 20 minutes (until the reaction mixture cooled to a temperature of about 130 degrees Fahrenheit) at which time the reaction to form this first solution was complete.

Example 10: Commercial Production of a Solubility Enhancing Composition Second Solution

To a one thousand gallon polyethylene conical-bottom tank is added deionized water equal to the volume or mass of the first solution. To this water is added the first solution. The resulting mixture represents a second solution of the present invention.

Example 11: Ion Chromatography Results

Using the sample preparations set forth in Example 9 and the ion chromatography methods set forth in Example 7, the following results (averages of 3 replicates of 3 samples) were obtained:

| Sulfate mol/L  | Ammonium mol/L |
|----------------|----------------|
| 10.77769681    | 1.677964718    |
| Target Ranges: |                |
| Sulfate mol/L  | Ammonium mol/L |
| 8.00-13.00     | 1.45-2.01      |

Example 12. Preparation of an Aqueous Paper Enhancing Composition (Also Used for the Preparation of an Aqueous Carbonate Enhancing Composition)

A 30% sodium hydroxide solution is prepared by dissolving 300 grams of sodium hydroxide per 1000 grams (1.0 L) of water;

A 50% Glucopon® 420 solution is prepared by dissolving 500 grams of Glucopon 420 per 1000 grams (1.0 L) of water;

38

To an appropriate mixing vessel is added 2700.98 grams of water; To the water is added 551.60 grams of a first solution (as defined above) with slow mixing; To the previous solution is added 276.91 grams of a 30% sodium hydroxide solution with slow mixing; Mix the previous solution slowly for 30 minutes and, after which, adjust the pH to 3.0; To the previous solution, slowly add 891.74 grams of copper sulfate with mixing until the copper sulfate is fully dissolved; To the previous solution, add 5.80 grams of 50% Glucopon 420 and mix for 1 hour; Adjust the final pH to 3.0 with sodium hydroxide.

Example 13. Commercial-Scale Preparation (330 Gallons of Finished Product) of an Aqueous Paper Enhancing Composition (Also Used for the Preparation of an Aqueous Carbonate Enhancing Composition)

To a 500 gallon polyethylene tank was added 2,116 pounds of 17 megohm water, with mixing via circulation from a roller pump; To the water was added 183 pounds of a solubility enhancing aqueous composition, with continued mixing; To the prior solution was slowly added 183 pounds of 50% sodium hydroxide, with continued mixing; To the prior solution was added 590 pounds of copper sulfate, with continued mixing to maintain the copper sulfate in solution; To the prior solution/suspension was added 2 pounds of Glucopon 420® with continued mixing for one hour pH of the final solution is adjusted to a pH from about 2.5 to about 3.5 using additional solubility enhancing aqueous composition when the pH needs to be lowered or add sodium hydroxide if the pH needs to be increased to the target range.

Example 14: The Following Antimicrobial Composition was Used for the Analysis in Example 15 and Antimicrobial Tests in Examples 16 and 17

Solubility enhancing aqueous composition: 0.9% w/w  
Dilute sodium hydroxide: 0.089% w/w  
Glucopon (50%): 0.06% w/w  
Silver sulfate: 0.022% w/w  
Water: 98.93% w/w

Example 15. Silver Quantification in an Antimicrobial Composition

Test samples were produced, and atomic absorption was performed for the quantification of silver. Briefly, samples were diluted 10:1 and run on a calibrated Thermo iCE 3500 flame atomic absorption spectrometer. Silver was measured at 140 ppm for a stock solution and additional dilutions were made to 35 ppm and 17.5 ppm and all were used for antimicrobial testing.

Example 16. Antibacterial 10-Minute Contact Time Testing

Overnight cultures of *Staphylococcus aureus*, *Pseudomonas aeruginosa*, and *Salmonella enterica* were produced in nutrient broth at 37° C. with gentle shaking.

39

For testing, nutrient agar plates were warmed to room temperature. Bacteria were washed once with sterile Butterfield phosphate, gently pelletized with a benchtop centrifuge, and resuspended in Butterfield phosphate.

500  $\mu$ l of test solution was added into 1.5 ml tubes 5 Butterfield phosphate was used as a

Control. 50  $\mu$ l of washed bacteria was added to each tube. Tubes were incubated 10 minutes.

At 10 min, tubes were spun down in a benchtop centrifuge 10 to pellet bacteria. Bacteria were resuspended in 500  $\mu$ l Butterfield phosphate. Serial dilutions were performed and plated onto nutrient agar plates. Plates were incubated overnight at 37°C.

All solutions produced greater than 5-log reductions in *S. aureus* at 10 minute contact times. The 35 ppm and 140 ppm 15 dilutions showed greater than 5-log reductions in *P. aeruginosa* and *S. enterica* at 10 minute contact times.

#### Example 17. Antibacterial Residual Efficacy Testing

Further experiments explored the feasibility of using 20 solutions as antibacterial surface treatments. Polystyrene (PS) petri dishes were used as test surfaces. Dishes were minimally swabbed with 140 ppm silver solution and allowed to dry overnight.

At 24 h post application, *S. aureus* and *P. aeruginosa* were swabbed into the plates. Control and test plates were allowed to fully dry (approx. 15 min).

1 mL of Butterfield phosphate was pipetted across the 25 plate repeatedly to rinse the plates and collected. Serial dilutions were made in Butterfield phosphate and plated on nutrient agar plates. Plates were incubated overnight at 37°C.

*S. aureus* growth was reduced by greater than 3-log. *P. aeruginosa* growth was reduced between 1- and 2-log.

#### Example 18: Sample Antimicrobial Composition

To 950 mL of deionized water is added 0.9 mL of a 30 solubility enhancing aqueous composition, 0.89 mL of a sodium hydroxide solution, 0.6 mL of Glucopon 420, and 0.22 g silver sulfate. Solution is stirred until the pH is stable. pH is adjusted to 4.5 using additional sodium hydroxide or sulfuric acid and the resultant solution is brought to 1000 mL total.

#### Example 19: Antiviral Activity on COVID-19 with Antimicrobial Compositions

Antimicrobial compositions of the present invention were 35 tested for hard surface efficacy (1 and 6 hours) by Microbac Laboratories, Inc. (Sterling, VA USA) for activity against SARS-CoV-2 (COVID-19 Virus Strain USA-WA1/2020 (source: BEI Resources, NR-52281).

Compositions used:

Water: 68.85%

Solubility Enhancing Aqueous Composition: 5.935%

Sodium Hydroxide: 5.96%

Glucopon: 0.07%

Copper Sulfate: 19.195%

Water: 3759.3 grams

Solubility Enhancing Aqueous Composition: 3.38 grams

50% Sodium Hydroxide: 3.4 grams

Glucopon: 2.5 grams

Silver Sulfate: 8.3 grams

Experimental design was:

Host Cell Line: Vero E6 cells, ATCC CRL-1585

40

Dilution Medium: Minimal Essential Medium (MEM)+Newborn Calf Serum (NCS) Neutralizer: MEM+10% NCS+0.5% Lecithin+1 mM EDTA

Contact Time: 1 and 6 hours

Contact Temperature: Room Temperature (20+1°C., Actual 20°C.)

Relative Humidity: 48% RH

Number of Replicates: 1 replicate (4 wells per dilution)

According to the U.S. Environmental Protection Agency, the test substance passes the Virucidal Hard-Surface Efficacy Test of the product demonstrates a  $\geq\log_{10}$  reduction on each surface in the presence or absence of cytotoxicity. When cytotoxicity is present, the virus control titer should be increased, if necessary, to demonstrate a  $\geq\log_{10}$  reduction in viral titer on each surface beyond the cytotoxic level.

Results:

Antimicrobial Composition with copper sulfate—1 hour: passed

Antimicrobial Composition with copper sulfate—6 hours: passed

Antimicrobial Composition with silver sulfate—1 hour: passed

Antimicrobial Composition with silver sulfate—6 hours: passed

#### Example 20: Further Explanation of Preparation of Test Compounds and Antimicrobial Activity

Atomic Absorption, using the method described herein, was initially performed for the quantification of silver in several samples. All samples contained between 560 and 94 ppm. Silver in Sample 1 was quantified at 140 ppm and was 35 selected, in addition to additional dilutions as set forth herein, for further antibacterial testing.

Initial experiments with Sample 1 focused on antibacterial capabilities in solution. *Staphylococcus aureus*, *Pseudomonas aeruginosa*, and *Salmonella enterica* were all challenged with full strength or dilutions of sample Sample 1. Bacteria were cultured in nutrient broth overnight at 37°C. to ensure log phase growth at time of testing. Treatments of Sample 1, in which bacteria culture was added to Sample 1 solution prior to plating on nutrient agar overnight at 37°C., ranged from full strength (140 ppm) to 8-fold (17.5 ppm) for *S. aureus*, and to 4-fold (35 ppm) for *P. aeruginosa* and *S. enterica*. Initial testing with *S. aureus* used a 10-minute and 45-minute incubation of bacteria in Sample 1 solution and further testing with other bacteria used a 10-minute incubation only.

50 Treatment of *S. aureus* in Sample 1 solution for as little as 10 minutes eliminated all viable bacteria diluted down to the lowest (8-fold) dilution. The lowest dilution used against *P. aeruginosa* and *S. enterica* (4-fold) was also successfully prohibited all growth.

55 For the sake of clarity, the 8-fold dilution of silver is equivalent to 0.002529% of silver sulfate in a composition described in Example 12 and in antimicrobial compositions as otherwise described herein; and the 4-fold dilution of silver is equivalent to 0.005058% of silver sulfate in a composition described in Example 12 and in antimicrobial compositions as otherwise described herein.

#### Example 21: Antibacterial Pretreatment of Polystyrene

60 Further experiments explored the feasibility of using Sample 1 as an antibacterial pretreatment of polystyrene

(PS) to control bacterial colonization and growth. PS plates were coated with full strength Sample 1 solution and allowed to dry overnight before *S. aureus* and *P. aeruginosa* were swabbed into the plates. Control and test plates were allowed to fully dry (approx. 15 min) before Butterfield Phosphate (BPS) buffer was used to rinse the plates and collected for agar plating. Log dilutions were made in BPS and allowed to grow on nutrient agar overnight at 37° C.

PS pretreatment with Sample 1 reduced *S. aureus* growth by greater than 3-log. *P. aeruginosa* growth was reduced between 1- and 2-log, indicating that Sample 1 may reduce overall bacterial colonization and growth but is a more effective pretreatment against *S. aureus*.

We claim:

1. A paper enhancing composition comprising: a solubility enhancing composition comprising an anionic component comprising sulfate ions, alone or in combination with bisulfate ions, having a concentration from about 8.00 moles per liter to about 13.00 moles per liter of the solubility enhancing composition volume, a cationic component comprising ammonium ions having a concentration from about 1.45 moles per liter to about 2.01 moles per liter of the solubility enhancing composition volume, and a hydrogen ion component in a concentration from about 17.38 to about 21.68 moles per liter of the total volume of the solubility enhancing composition;

a dilute sodium hydroxide solution having a concentration of about 5 percent to about 7.5 percent weight/weight of the total aqueous phase weight of the paper enhancing composition wherein the dilute sodium hydroxide solution has a concentration from about 20 percent to about 50 percent sodium hydroxide; and

silver sulfate having a concentration from about 0.001 percent to about 1.5 percent weight/weight of the total weight of the paper enhancing composition.

2. The paper enhancing composition of claim 1 further comprising at least one surfactant selected from the group consisting of non-ionic surfactant and anionic surfactant having a concentration from about 0.05 percent to about 0.15 percent weight/weight of the total aqueous phase weight of the paper enhancing composition.

3. The paper enhancing composition of claim 1 further comprising the addition of at least one acid or at least one base to adjust the final pH of the paper enhancing composition in a range from about pH 2.5 to about pH 3.5.

4. The paper enhancing composition of claim 2 further comprising the addition of at least one acid or at least one base to adjust the final pH of the paper enhancing composition in a range from about pH 2.5 to about pH 3.5.

5. The paper enhancing composition of claim 3, wherein the paper enhancing composition is substantially free of solids.

6. The paper enhancing composition of claim 4, wherein the paper enhancing composition is substantially free of solids.

7. The paper enhancing composition of claim 3, wherein the paper enhancing composition is free of solids.

8. The paper enhancing composition of claim 4, wherein the paper enhancing composition is free of solids.

9. A paper enhancing composition consisting of: a solubility enhancing composition comprising an anionic component comprising sulfate ions, alone or in combination with bisulfate ions, having a concentration from about 8.00 moles per liter to about 13.00 moles per liter of the solubility enhancing composition volume, a cationic component comprising ammonium ions having a concentration from about 1.45 moles per liter to about 2.01 moles per liter of the solubility enhancing composition volume, and a hydrogen ion component in a concentration from about 17.38 to about 21.68 moles per liter of the total volume of the solubility enhancing composition;

a dilute sodium hydroxide solution having a concentration of about 5 percent to about 7.5 percent weight/weight of the total aqueous phase weight of the paper enhancing composition wherein the dilute sodium hydroxide solution has a concentration from about 20 percent to about 50 percent sodium hydroxide;

at least one surfactant selected from the group consisting of non-ionic surfactant and anionic surfactant having a concentration from about 0.05 percent to about 0.15 percent weight/weight of the total aqueous phase weight of the paper enhancing composition;

silver sulfate having a concentration from about 0.001 percent to about 1.5 percent weight/weight of the total weight of the paper enhancing composition; and at least one acid or at least one base to adjust the final pH of the paper enhancing composition in a range from about pH 2.5 to about pH 3.5.

10. The paper enhancing composition of claim 9, wherein the paper enhancing composition is substantially free of solids.

11. The paper enhancing composition of claim 9, wherein the paper enhancing composition is free of solids.

12. A solubility enhancing aqueous composition comprising an anionic component comprising sulfate ions, alone or in combination with bisulfate ions, having a concentration from about 8.00 moles per liter to about 13.00 moles per liter of the solubility enhancing composition volume, a cationic component comprising ammonium ions having a concentration from about 1.45 moles per liter to about 2.01 moles per liter of the solubility enhancing composition volume, and a hydrogen ion component in a concentration from about 17.38 to about 21.68 moles per liter of the total volume of the solubility enhancing composition solution.

\* \* \* \* \*